

## 1

2,892,704

## TITANIUM BASE ALLOYS

Robert I. Jaffee, Worthington, and Horace R. Ogden and Daniel J. Maykuth, Columbus, Ohio, assignors, by mesne assignments, to Crucible Steel Company of America, Flemington, N.J., a corporation of New Jersey

No Drawing. Application July 9, 1956  
Serial No. 596,459

## 1 Claim. (Cl. 75—175.5)

This invention pertains to improvements in titanium base alloys, and provides a series of alloys of high strength and ductility, and, as to certain analyses, also of high contamination resistance and high strength at elevated temperatures, and containing as essential constituents titanium and tin, together with one or more additional metals selected from the groups comprising alpha promoters, beta promoters and compound formers as enumerated below.

This application is a continuation-in-part of our applications Serial Nos. 285,076, filed April 29, 1952, now U.S. Letters Patent No. 2,669,513, dated February 16, 1954; 294,262 and 294,263, both filed June 18, 1952, and both now abandoned; 344,686, filed March 25, 1953, now abandoned; and 396,756, filed December 7, 1953, now Patent No. 2,797,996, granted July 2, 1957.

The tin content may be present over a broad range of about 0.5 to 23%, with a preferred lower limit of about 2.5%, as adjudged from the standpoint of good room temperature mechanical properties, and a preferred lower limit of about 5% as regards the imparting of high contamination resistance at elevated temperatures. To the titanium-tin alloy aforesaid, there may advantageously be added up to about 18% in aggregate of one or more of the alpha promoters, up to about 50% in aggregate of one or more of certain of the beta promoters, and up to about 2 or 3% in aggregate of the compound formers, all as set forth more in detail hereinafter. For further enhancing the mechanical properties, the alloys of the invention may contain controlled amounts of the interstitials, carbon, oxygen and nitrogen. For certain analyses, as set forth below, carbon may be present up to about 1%, oxygen up to about 0.5% and nitrogen up to about 0.4%. For a tin content below about 5%, and particularly below about 2.5%, substantial additions of one or more of the interstitials carbon, oxygen and nitrogen or of metal of the alpha and/or beta promoter groups, is required for imparting adequate tensile properties for commercial applications, as elaborated upon below.

As above stated, the alloys of the invention are in general characterized by excellent room temperature mechanical properties, possessing high tensile strength as compared to the unalloyed titanium base metal, combined with adequate ductility for both hot and cold forming operations, i.e., forging, rolling, drawing, extruding, etc. For tin contents up to about 16%, they may likewise, in general, be welded without appreciable loss of ductility in the welded as compared to the non-welded portions. This is particularly true as regards those alloys having an all-alpha microstructure, and also as to certain of those having a beta-containing microstructure, as explained more in detail below.

## 2

For imparting a high degree of contamination resistance, i.e., resistance against penetration by atmospheric gases, particularly oxygen and nitrogen, at elevated temperatures up to about 1100° C., the alloys should contain upwards of about 5% tin, although lesser amounts down to about 2% tin are materially beneficial in this respect. Tin alloyed with titanium base metal appears to be unique in imparting this contamination resistance, and its effect is quite critical with respect to the degree of contamination resistance imparted commencing at a minimum of about 5% tin.

These contamination resistant alloys are also characterized by free scaling properties resulting from exposure to elevated temperatures up to about 1100° C. and to atmospheric, oxidizing, or alternately oxidizing and reducing conditions. That is to say, the scale formed is easily brushed off or flakes off during hot forming operations, such as forging or rolling.

As is known, the metal titanium in the pure state, is capable of existing in either of two allotropic forms. Below a temperature of about 885° C. or 1625° F., it assumes a close-packed hexagonal structure known as the alpha phase, while at this temperature and above it assumes a body-centered cubic structure known as the beta phase.

Certain substitutional alloying additions to the titanium base metal, among which may be mentioned tin, antimony, indium, silver, bismuth, lead, cadmium, zinc, and thallium as well as the interstitials carbon, oxygen, and nitrogen may be termed alpha stabilizers or alpha promoters. The term alpha stabilizer includes those elements which raise the transformation range sharply, such as oxygen and nitrogen. Also alpha stabilizers include elements such as carbon, which have a relatively small solubility in alpha titanium, but which raise the transformation temperature for that amount which is in solution. Alpha stabilizers also include those elements such as tin, antimony, indium, and silver which have relatively large solubilities, of about the same magnitude, in both the alpha and beta phases and which have little effect on the transformation temperature range, neither raising nor lowering it markedly. A common characteristic of the alpha stabilizers, as we are considering them here, is that little or no hardening occurs in the thermal processing. The resulting alloys are, at room temperature, always all alpha in structure regardless of the heat treatment, including quenching or aging. Actually little is known concerning the specific effects of bismuth, lead, cadmium, zinc, and thallium on the transformation range. These alloying elements produce alloys which fit the criteria given, namely, that they form all-alpha alloys, which do not retain any substantial content of beta phase nor harden appreciably on quenching from the beta field. Hence these elements appear properly classified as alpha promoters, and will be so treated in this application.

Other substitutional alloying elements, when added in progressively increasing quantities, stabilize the beta phase at progressively lower temperatures, until a mixed alpha-beta or stable all-beta microstructure is obtained at normal or atmospheric temperatures, or the beta phase undergoes a eutectoid reaction, depending on the character and amount of the beta stabilizers added as discussed below.

Speaking in broadest terms, the beta stabilizers are Mo, V, Cr, Ta, Zr, Mn, Cr, Fe, W, Ni, Co and Cu.

Silicon and beryllium may also be considered as beta stabilizing elements, but their solubilities in titanium are relatively so slight and the tendency of the beta phase stabilized by these elements to decompose into eutectoid products so great, that it is equally proper to consider them as compound-forming elements. Within this broad category, however, only certain of the elements mentioned are suitable for producing mixed-phase, alpha-beta alloys, or all-beta alloys. These are the elements which have beta-isomorphous diagrams, or which have beta-eutectoid diagrams such that the decomposition of the beta phase into eutectoid is so sluggish that the alloys behave like those in a beta-isomorphous system. The beta stabilizing elements of this type are Mo, V, Cb, Ta, Mn, Fe and Cr. Tungsten is a borderline element as between the sluggishly decomposing and rapidly decomposing types and hence may be classified either way. Within this limited group only Mo, V, Cb and Ta are beta-isomorphous. They form the most thermally stable beta-containing alloys, as a result of their beta-isomorphism.

Zirconium is a beta promoter or stabilizer in the sense that the lowest temperature at which alloys thereof with titanium are entirely beta, becomes progressively lower with increasing amounts of zirconium, until a composition is reached at which this so-called beta transus temperature starts to increase again with further additions of zirconium. While zirconium thus lowers the transformation temperature of titanium, the alloys eventually revert to the alpha phase at lower temperatures unless other beta-promoters are present. Zirconium is isomorphous with titanium both in the alpha and beta fields. As a result, it is proper to consider zirconium together with vanadium, molybdenum, columbium and tantalum as all being beta-isomorphous with titanium.

The use of copper alone as an alloying addition to titanium, does not fit into the above-mentioned grouping of beta-isomorphous and sluggishly decomposing eutectoid beta promoters, because the beta phase stabilized by copper always decomposes rather rapidly into proeutectoid and eutectoid products, and the same is generally true with respect to cobalt, nickel, silicon and beryllium, above listed under the broad category of beta stabilizers. Copper, however, is a useful addition when present as a minor alloying element, for example, up to a few percent, in alloys containing larger amounts of other beta-stabilizing elements, within the narrow group of elements last mentioned above since, in these low concentrations and in the presence of such other beta-stabilizing elements, the tendency of the beta phase stabilized in part by copper to decompose into eutectoid products is minimized or entirely eliminated.

The tolerance of the ductile Ti-Sn base alloys of the invention with respect to additions of the various beta-promoters above mentioned, varies considerably for the individual elements of the group, being greatest with respect to those which form beta-isomorphous systems with titanium, and least for those which decompose most readily into eutectoid decomposition products. Thus, the Ti-Sn base alloys may be strengthened without undue embrittlement by additions of up to about 50% in aggregate of elements composing the beta-isomorphous group, viz., molybdenum, vanadium, columbium, tantalum and zirconium, since these elements are soluble in all proportions in beta titanium. Of the sluggishly decomposing elements, the base alloy will tolerate additions of up to about 20% of either or both chromium and tungsten, up to about 10% manganese, and up to about 7% iron. Copper may be added up to about 7%. Metal of the group cobalt and nickel may be added up to a total of about 5%. For additions of all of the above-mentioned beta-promoters, the lower effective limit is about 0.5% and preferably about 1%.

The tolerance of the ductile Ti-Sn base alloys for

the alpha promoters depends on the amount of tin present, the less tin present the greater the amount of alpha-promoters that can be added and vice versa. Antimony may be added to a maximum content of 18%. The proportioning of antimony content in relation to the tin content is given below. Indium may be added up to a maximum content of 15%. Silver may be added up to about 20%. Cadmium, zinc, thallium, bismuth and lead may be added up to 15% each, added to the charge in melting. The lower effective limit for the alpha promoters is about 0.5% and preferably about 1%.

The elements Ce, Be, As, S, Te and P are strictly compound-forming elements. They do not have appreciable solubilities in either the alpha or beta phases, but form intermetallic compounds with titanium. The beta promoters silicon and beryllium are likewise best grouped as compound-forming elements, in view of their above-mentioned low solubilities in titanium and the tendency of the beta phase stabilized by these elements to decompose rapidly into eutectoid products. The Ti-Sn alloys of the invention will tolerate only relatively small amounts of these compound-forming elements, i.e., up to a total of about 2 or 3% maximum, the lower effective limit being about 0.1 or 0.2%.

Substantially pure and ductile metallic titanium may be produced at considerable expense by the so-called "iodide" process described in U.S. Patent 1,671,213 to Van Arkel; while ductile titanium of commercial purity is produced more cheaply by the magnesium reduction of titanium tetrachloride by the process described in U.S. Patent 2,205,854 to Kroll. Both procedures, particularly the latter, result in some contamination of the titanium metal with one or more of the interstitials, carbon, oxygen and nitrogen. But since, as noted above, these are all alpha-promoting or stabilizing elements, the resultant somewhat contaminated titanium metal obtained, has at room temperatures a single phase, all-alpha microstructure.

The all-alpha, all-beta and mixed alpha-beta alloys of titanium have their respective advantages and disadvantages. Generally speaking, the alpha alloys provide good all-around performance, having good weldability, and being strong and resistant to oxidation, both cold and hot, but are somewhat inferior as to ductility. The all-beta alloys, on the other hand, have excellent bendability and ductility, are strong both hot and cold, but are somewhat vulnerable to atmospheric contamination, particularly at elevated temperatures. The mixed alpha-beta alloys provide a compromise performance as between all-alpha and all-beta alloys, being strong when cold and warm, but weak hot, while possessing good bendability and ductility, with a moderate degree of resistance to atmospheric contamination.

Since the Ti-Sn base alloys have, as above noted, an all-alpha microstructure, they may be readily welded in tin contents up to about 16%, with no appreciable impairment of ductility in the welded as compared to the non-welded portions. They also form an excellent base alloy for the ternary and higher component alloys of the invention, that may be also welded without appreciable loss of ductility in the welded as compared to the non-welded portions. This is particularly true as regards the above-mentioned alpha-promoter additions to the base alloy. Also, in general, the ternary and higher component alloys made by additions of the beta-isomorphous elements above designated are weldable without appreciable impairment of ductility. It may furthermore be stated that in general the alpha-beta alloys according to the invention can be produced to have ductile welded portions if suitable post-welding heat treatments are applied as described in the co-pending application of Jaffee et al., Serial No. 585,177, filed May 16, 1956, which is a continuation-in-part of application Serial No. 305,504, filed August 20, 1952 and now abandoned.

Antimony is a particularly valuable addition to the titanium-tin base metal as it imparts about the same strengthening effect as equivalent additions of tin. As the tin content increases, the tolerance for antimony decreases and vice versa with respect to retention of adequate ductility, in accordance with the following tabulation:

| Percent Tin | Percent Antimony, Max. |
|-------------|------------------------|
| 1           | 17                     |
| 5           | 15                     |
| 10          | 10                     |
| 17.5        | 5                      |
| 23          | 0.5                    |

Tin is soluble in alpha titanium to the extent of at least 15%, and alloys of titanium with up to 15% tin are all in the alpha phase. As the tin content is increased, the beta transformation temperature rises, and at a temperature of about 930° C., and a tin content of about 19%, a peritectoid reaction occurs. In alloys containing about 20 to 23% tin, two intermediate phases formed at different temperatures have been tentatively identified.

- 10 The following Table I gives, for comparative purposes with the further test data presented hereinafter, test results showing the improvement in mechanical properties, resulting from additions of tin over the range of about 1 to 23%, to both "iodide" and "commercial purity" 15 titanium base metal, with and without further controlled additions of one or more of the interstitials, carbon, oxygen and nitrogen:

TABLE I

## Ti-Sn binary alloys

[Annealed condition.]

| Composition, Percent<br>(Balance Titanium) |      |      |      | Tensile Properties:<br>p.s.i. $\times 1,000$ |                      | Percent<br>Elonga-<br>tion in 1" | Percent<br>Reduct-<br>tion in<br>Area | Vickers<br>Hard-<br>ness | Min.<br>Bend<br>T |
|--------------------------------------------|------|------|------|----------------------------------------------|----------------------|----------------------------------|---------------------------------------|--------------------------|-------------------|
| Sn                                         | C    | O    | N    | 0.2%<br>Offset<br>Yield                      | Ultimate<br>Strength |                                  |                                       |                          |                   |
| IODIDE TITANIUM BASE                       |      |      |      |                                              |                      |                                  |                                       |                          |                   |
| 0                                          |      |      |      | 27                                           | 43                   | 40                               | 61                                    | 105                      | 0                 |
| 2.5                                        |      |      |      | 50                                           | 69                   | 23                               | 50                                    | 217                      | 0.9               |
| 5                                          |      |      |      | 66                                           | 78                   | 26                               | 37                                    | 235                      | 1.6               |
| 10                                         |      |      |      | 85                                           | 99                   | 20                               | 36                                    | 298                      | 1.5               |
| 15                                         |      |      |      | 98                                           | 110                  | 19                               | 35                                    | 320                      | 1.5               |
| 20                                         |      |      |      | 117                                          | 122                  | 12                               | 36                                    | 324                      | 1.5               |
| 22.5                                       |      |      |      | 135                                          | 149                  | 11                               | 19                                    | 339                      | 4.7               |
| 1                                          | 0.2  |      |      | 55                                           | 70                   | 28                               | 48                                    | 205                      | 0                 |
| 2.5                                        | 0.2  |      |      | 65                                           | 74                   | 29                               | 51                                    | 235                      | 0.5               |
| 5                                          | 0.2  |      |      | 79                                           | 88                   | 29                               | 53                                    | 265                      | 0.5               |
| 5                                          | 0.5  |      |      | 109                                          | 117                  | 24                               | 43                                    | 325                      | 1.3               |
| 4                                          | 1    |      |      | 123                                          | 138                  | 7                                | 13                                    | 387                      | 8.6               |
| 10                                         | 0.2  |      |      | 97                                           | 102                  | 24                               | 60                                    | 308                      | 1.0               |
| 10                                         | 0.5  |      |      | 130                                          | 147                  | 17                               | 51                                    | 373                      | 2.1               |
| 15                                         | 0.2  |      |      | 122                                          | 127                  | 11                               | 32                                    | 364                      | 1.6               |
| 1                                          |      | 0.2  |      | 64                                           | 84                   | 25                               | 38                                    | 237                      | 2.0               |
| 2.5                                        |      | 0.2  |      | 71                                           | 90                   | 24                               | 33                                    | 274                      | 2.0               |
| 5                                          |      | 0.2  |      | 79                                           | 96                   | 23                               | 47                                    | 312                      | 1.0               |
| 5                                          |      | 0.5  |      | 128                                          | 128                  | 1                                | 10                                    | 423                      | 7.6               |
| 10                                         |      | 0.2  |      | 99                                           | 112                  | 16                               | 32                                    | 360                      | 1.7               |
| 10                                         |      | 0.4  |      | 131                                          | 138                  | 1                                | 23                                    | 410                      | 6.5               |
| 15                                         |      | 0.3  |      | 124                                          | 134                  | 20                               | 40                                    | 380                      | 2.3               |
| 15                                         |      | 0.5  |      | 147                                          | 155                  | 11                               | 38                                    | 300                      | 3.2               |
| 1                                          |      |      | 0.2  | 94                                           | 105                  | 14                               | 33                                    | 310                      | 2.0               |
| 2.5                                        |      |      | 0.2  | 100                                          | 109                  | 16                               | 26                                    | 332                      | 1.7               |
| 5                                          |      |      | 0.11 | 80                                           | 97                   | 19                               | 29                                    | 296                      | 2.0               |
| 5                                          |      |      | 0.29 | 120                                          | 123                  | 20                               | 47                                    | 348                      | 2.8               |
| 10                                         |      |      | 0.11 | 88                                           | 100                  | 18                               | 32                                    | 297                      | 2.1               |
| 10                                         |      |      | 0.27 | 128                                          | 134                  | 18                               | 46                                    | 364                      | 2.2               |
| 15                                         |      |      | 0.30 | 146                                          | 154                  | 12                               | 38                                    | 397                      | 2.9               |
| COMMERCIAL PURITY TITANIUM BASE            |      |      |      |                                              |                      |                                  |                                       |                          |                   |
| 0                                          |      |      |      | 51                                           | 76                   | 21                               | 51                                    | 201                      | 0.8               |
| 1                                          |      |      |      | 48                                           | 73                   | 21                               | 54                                    | 198                      | 0.8               |
| 2.5                                        |      |      |      | 67                                           | 86                   | 14                               | 48                                    | 236                      | 1.5               |
| 5                                          |      |      |      | 71                                           | 90                   | 14                               | 42                                    | 246                      | 1.5               |
| 10                                         |      |      |      | 91                                           | 110                  | 11                               | 36                                    | 296                      | 1.5               |
| 15                                         |      |      |      | 108                                          | 123                  | 10                               | 35                                    | 313                      | 2.3               |
| 20                                         |      |      |      | 128                                          | 131                  | 10                               | 39                                    | 330                      | 2.2               |
| 22.5                                       |      |      |      | 139                                          | 150                  | 5                                | 19                                    | 341                      | 2.2               |
| 5                                          | 0.17 |      |      | 98                                           | 106                  | 27                               | 61                                    | 311                      | 1.8               |
| 4                                          | 0.4  |      |      | 113                                          | 121                  | 26                               | 60                                    | 335                      | 1.8               |
| 5                                          | 0.96 |      |      | 121                                          | 129                  | 7                                | 11                                    | 367                      | 3.0               |
| 5                                          |      | 0.2  |      | 109                                          | 123                  | 24                               | 53                                    | 351                      | 2.5               |
| 5                                          |      | 0.4  |      | 137                                          | 148                  | 8                                | 10                                    | 403                      | Brittle           |
| 5                                          |      | 0.28 |      | 142                                          | 149                  | 12                               | 31                                    | 388                      | 7.4               |
| 5                                          |      | 0.42 |      | 159                                          | 164                  | 1                                | 8                                     | 415                      | Brittle           |
| 10                                         | 0.2  |      |      | 112                                          | 118                  | 26                               | 53                                    | 356                      | 1.9               |
| 10                                         | 0.58 |      |      | 146                                          | 148                  | 11                               | 32                                    | 385                      | 4.5               |
| 13                                         | 0.1  |      |      | 109                                          | -----                | 19                               | 45                                    | -----                    | 1.8               |
| 10                                         |      | 0.2  |      | 122                                          | 131                  | 19                               | 44                                    | 358                      | 2.8               |
| 10                                         |      | 0.4  |      | 131                                          | 138                  | 16                               | 39                                    | 386                      | 3.3               |
| 10                                         |      | 0.13 |      | 114                                          | 124                  | 18                               | 45                                    | 337                      | 1.7               |
| 16                                         | 0.2  |      |      | 114                                          | 139                  | 14                               | 27                                    | 337                      | 2.1               |
| 16                                         |      | 0.2  |      | 109                                          | 137                  | 12                               | 22                                    | 341                      | 3.3               |
| 16                                         |      | 0.18 |      | 128                                          | 149                  | 9                                | 16                                    | 331                      | 6.1               |
| 19                                         | 0.2  |      |      | 140                                          | 158                  | 9                                | 15                                    | 357                      | 4.0               |
| 19                                         |      | 0.2  |      | 120                                          | 140                  | 18                               | 33                                    | 339                      | 2.1               |
| 19                                         |      | 0.14 |      | 127                                          | 151                  | 5                                | 22                                    | 357                      | 4.2               |

From these results it will be observed that additions of tin up to about 23% greatly strengthens the metal while retaining adequate ductility for fabrication purposes, i.e., forging, rolling, etc. For the "iodide" titanium base the yield strength is more than quadrupled from 27,000 to 135,000 p.s.i., while the ultimate strength is more than tripled from 43,000 to 149,000 p.s.i. For any given tin content further strengthening results from controlled additions of one or more of the interstitials. Thus, at the 5% tin level, the addition of 0.5% carbon, 10 approximately doubles the yield and ultimate strength without reducing ductility. Oxygen and nitrogen additions have generally similar effects as shown. In this way the tensile strength of the material may be raised to as much as about 160,000 p.s.i. with retention of adequate ductility as shown, for example, by the 19% tin, 0.2% carbon, commercial purity base analysis.

Considering now the strengthening effects of additions to the titanium-tin base alloys as typified by Table I, of one or more of the alpha promoters, beta promoters, or compound formers above discussed, the following Table II gives test results for additions of one of the more important beta promoters, namely, manganese:

of ductility. In fact, for additions of manganese up to about 6%, the ductility is actually increased as compared to the alloy omitting manganese, while at the same time, increasing the ultimate strength up to about 150,000 p.s.i. The effect of interstitial additions to the manganese-containing alloy again enhances the strength without serious effect on ductility as shown by comparison of the 9% tin, 2.5% and 5% Mn analyses.

The following Tables III and IV show the effects of molybdenum additions to the titanium-tin base alloy. In Table III all alloys are in the annealed condition; whereas Table IV gives the properties of the alloys in various heat treated conditions. Here again, as in the case of manganese, the molybdenum additions greatly increase the strength of the alloy while retaining adequate ductility. For example, with the 10% tin analysis and a 7.5% molybdenum addition, the ultimate strength is increased from 110,000 to 140,000 p.s.i. with no loss in ductility, as shown by comparison with Table I. At the 15% tin level the ultimate strength is increased from 123,000 to 167,000 p.s.i. with no loss in ductility upon the addition of 5% molybdenum. The effect of adding interstitials

TABLE II  
Ti—Sn—Mn alloys (commercial titanium base)  
[Annealed condition.]

| Composition, Percent (Balance Titanium) |      |      |     |      | Tensile Properties:<br>p.s.i. $\times 1,000$ |                      | Percent<br>Elongation<br>in 1" | Percent<br>Reduction<br>in Area | Vickers<br>Hardness | Min.<br>Bend T |
|-----------------------------------------|------|------|-----|------|----------------------------------------------|----------------------|--------------------------------|---------------------------------|---------------------|----------------|
| Sn                                      | Mn   | O    | O   | N    | 0.2% Offset<br>Yield                         | Ultimate<br>Strength |                                |                                 |                     |                |
| 9                                       | —    | —    | —   | —    | 74                                           | 89                   | 21                             | 50                              | 276                 | 1.7            |
| 9                                       | 0.25 | —    | —   | —    | 72                                           | 90                   | 20                             | 48                              | 261                 | 1.6            |
| 9                                       | 0.5  | —    | —   | —    | 74                                           | 95                   | 24                             | 49                              | 273                 | 1.7            |
| 9                                       | 0.5  | 0.25 | —   | —    | 113                                          | 122                  | 20                             | 55                              | 369                 | 1.5            |
| 9                                       | 0.5  | —    | 0.2 | —    | 96                                           | 117                  | 20                             | 45                              | 364                 | 1.6            |
| 9                                       | 0.5  | —    | —   | 0.11 | 95                                           | 105                  | 20                             | 46                              | 344                 | 1.5            |
| 9                                       | 2.5  | —    | —   | —    | 107                                          | 118                  | 11                             | 46                              | 336                 | 1.2            |
| 9                                       | 2.5  | 0.2  | —   | —    | 138                                          | 143                  | 19                             | 39                              | 369                 | 1.8            |
| 9                                       | 2.5  | —    | 0.2 | —    | 135                                          | 144                  | 17                             | 39                              | 389                 | 1.8            |
| 9                                       | 2.5  | —    | —   | 0.2  | 143                                          | 150                  | 13                             | 46                              | 397                 | 2.8            |
| 9                                       | 5    | —    | —   | —    | 130                                          | 140                  | 16                             | 90                              | 353                 | 1.7            |
| 9                                       | 5    | 0.2  | —   | —    | 153                                          | 157                  | 16                             | 37                              | 424                 | 4.7            |
| 9                                       | 5    | —    | 0.2 | —    | 151                                          | 156                  | 14                             | 36                              | 421                 | 4.8            |
| 9                                       | 5    | —    | —   | 0.2  | 146                                          | 153                  | 12                             | 38                              | 426                 | 2.3            |
| 9                                       | 7.5  | —    | —   | —    | 120                                          | 129                  | 10                             | 11                              | 360                 | 1.6            |
| 10                                      | —    | —    | —   | —    | 91                                           | 110                  | 11                             | 36                              | 296                 | 1.5            |
| 10                                      | 1    | —    | —   | —    | 110                                          | 118                  | 12                             | 44                              | 341                 | 1.6            |
| 10                                      | 2    | —    | —   | —    | 121                                          | 128                  | 15                             | 48                              | 326                 | 1.7            |
| 10                                      | 3    | —    | —   | —    | 132                                          | 141                  | 15                             | 51                              | 356                 | 1.4            |
| 10                                      | 4    | —    | —   | —    | 129                                          | 140                  | 15                             | 39                              | 363                 | 1.6            |
| 10                                      | 5    | —    | —   | —    | 135                                          | 144                  | 12                             | 25                              | 375                 | 1.4            |
| 10                                      | 6    | —    | —   | —    | 144                                          | 151                  | 16                             | 38                              | 369                 | 1.4            |
| 10                                      | 7    | —    | —   | —    | 143                                          | 147                  | 9                              | 35                              | 386                 | 1.2            |
| 10                                      | 8    | —    | —   | —    | 161                                          | 164                  | 9                              | 27                              | 386                 | 2.9            |
| 10                                      | 9    | —    | —   | —    | 154                                          | 157                  | 10                             | 29                              | 377                 | 3.7            |
| 10                                      | 12   | —    | —   | —    | 171                                          | 173                  | 2                              | Br                              | 404                 | Br             |
| 1                                       | 5    | —    | —   | —    | 97                                           | 111                  | 20                             | 49                              | 316                 | 0.8            |
| 5                                       | 5    | —    | —   | —    | 116                                          | 126                  | 14                             | 41                              | 324                 | 1.6            |
| 15                                      | 5    | —    | —   | —    | 160                                          | 170                  | 4                              | 15                              | 431                 | 7.0            |

Comparing the results of the above table with those given in Table I, it will be seen, for example, that for the 10% tin alloy containing no manganese, the ultimate strength is 110,000 p.s.i., as compared to progressive increases ranging up to about 160,000 p.s.i. with additions of manganese up to about 9%, without serious impairment

70 is shown by comparison of the values for the 9% tin, 2.5% molybdenum analysis wherein the ultimate strength is increased from 113,000 to the order of 130,000 to 140,000 p.s.i. with no appreciable effect on ductility. The same order of increase occurs at the 9% tin, 5% molybdenum level.

TABLE III

## Ti—Sn—Mo alloys

[Annealed condition.]

| Composition, Percent<br>(Balance Titanium) |      |       | Tensile Properties:<br>p.s.i. $\times 1,000$ |                      | Percent<br>Elonga-<br>tion in 1" | Percent<br>Reduction<br>in Area | Vickers<br>Hardness | Min.<br>Bend T |
|--------------------------------------------|------|-------|----------------------------------------------|----------------------|----------------------------------|---------------------------------|---------------------|----------------|
| Sn                                         | Mo   | Other | 0.2% Off-<br>set Yield                       | Ultimate<br>Strength |                                  |                                 |                     |                |
| IODIDE TITANIUM BASE                       |      |       |                                              |                      |                                  |                                 |                     |                |
| 5                                          | —    | —     | 56                                           | 73                   | 26                               | 37                              | 235                 | 1.6            |
| 5                                          | 2.5  | —     | 68                                           | 91                   | 17                               | 41                              | 223                 | 1.0            |
| 10                                         | —    | —     | 84                                           | 101                  | 18                               | 44                              | 261                 | 2.0            |
| 15                                         | 2.5  | —     | 120                                          | 134                  | 9                                | 22                              | 304                 | 1.6            |
| COMMERCIAL TITANIUM BASE                   |      |       |                                              |                      |                                  |                                 |                     |                |
| 1                                          | 5    | —     | 101                                          | 105                  | 18                               | 64                              | 268                 | 1.0            |
| 5                                          | 5    | —     | 101                                          | 119                  | 18                               | 53                              | 290                 | 1.2            |
| 9                                          | 0.25 | —     | 78                                           | 96                   | 22                               | 52                              | 308                 | 1.6            |
| 9                                          | 0.5  | —     | 90                                           | 105                  | 19                               | 50                              | 300                 | 1.6            |
| 9                                          | 2.5  | —     | 96                                           | 113                  | 16                               | 45                              | 299                 | 1.7            |
| 9                                          | 5    | —     | 104                                          | 116                  | 14                               | 40                              | 313                 | 1.7            |
| 9                                          | 7.5  | —     | 43                                           | 130                  | 10                               | 17                              | 284                 | 1.7            |
| 9                                          | 10   | —     | 114                                          | 134                  | 15                               | 38                              | 302                 | 0.8            |
| 9                                          | 15   | —     | 121                                          | 124                  | 18                               | 38                              | 298                 | 0.8            |
| 10                                         | —    | —     | 91                                           | 110                  | 11                               | 36                              | 296                 | 1.5            |
| 10                                         | 7.5  | —     | 132                                          | 140                  | 9                                | 46                              | 314                 | 1.1            |
| 10                                         | 10   | —     | 135                                          | 142                  | 8                                | 26                              | 329                 | 0.2            |
| 15                                         | 5    | —     | 162                                          | 167                  | 7                                | 30                              | 362                 | 1.8            |
| 9                                          | 0.25 | 0.25O | 113                                          | 121                  | 25                               | 59                              | 352                 | 2.3            |
| 9                                          | 0.25 | 0.20  | 111                                          | 128                  | 23                               | 45                              | 378                 | 1.6            |
| 9                                          | 0.25 | 0.17N | 123                                          | 134                  | 19                               | 51                              | 366                 | 2.3            |
| 9                                          | 0.5  | 0.25O | 104                                          | 122                  | 23                               | 57                              | 369                 | 1.5            |
| 9                                          | 0.5  | 0.20  | 114                                          | 131                  | 22                               | 52                              | 364                 | 1.6            |
| 9                                          | 0.5  | 0.14N | 115                                          | 129                  | 19                               | 46                              | 392                 | 2.3            |
| 9                                          | 2.5  | 0.20  | 120                                          | 127                  | 14                               | 45                              | 343                 | 1.4            |
| 9                                          | 2.5  | 0.20  | 136                                          | 142                  | 11                               | 38                              | 375                 | 1.7            |
| 9                                          | 2.5  | 0.2N  | 135                                          | 145                  | 14                               | 38                              | 365                 | 1.8            |
| 9                                          | 5    | 0.20  | 137                                          | 140                  | 10                               | 30                              | 368                 | 2.5            |
| 9                                          | 5    | 0.20  | 133                                          | 142                  | 15                               | 33                              | 364                 | 2.5            |
| 9                                          | 5    | 0.2N  | 138                                          | 146                  | 9                                | 31                              | 364                 | 2.5            |
| 0.5                                        | 30   | —     | 140                                          | 141                  | 5                                | 17                              | 301                 | 1.0            |

TABLE IV

## Ti—Sn—Mo alloys

| Composition, percent<br>(Balance Titanium) | Condition               | Tensile Properties:<br>p.s.i. $\times 1,000$ |              | Percent<br>Elonga-<br>tion in 1" | Percent<br>Reduction<br>in Area | VHN | MBR, T |     |
|--------------------------------------------|-------------------------|----------------------------------------------|--------------|----------------------------------|---------------------------------|-----|--------|-----|
|                                            |                         | 0.2% Off-<br>set Yield                       | Ult.<br>Str. |                                  |                                 |     | L      | T   |
| 5Sn—6Mo                                    | Annealed                | 102                                          | 124          | 8                                | 28                              | —   | —      | —   |
| 5Sn—6Mo                                    | do                      | 107                                          | 125          | 16                               | 37                              | 300 | 1.4    | 2.8 |
| 5Sn—6Mo                                    | 1,600° F.—quenched      | 88                                           | 121          | 12                               | 15                              | 305 | 0      | —   |
| 5Sn—22.6Mo                                 | do                      | 117                                          | 129          | 8                                | 26                              | 322 | 1.3    | 1.2 |
| 6Sn—6Mo                                    | do                      | 81                                           | 123          | 14                               | 23                              | 295 | 0      | —   |
| 9Sn—6Mo                                    | do                      | 74                                           | 125          | 13                               | 14                              | 294 | 0      | —   |
| 4Sn—8Mo                                    | do                      | 66                                           | 127          | 16                               | 12                              | 320 | 4.0    | 9.0 |
| 4Sn—10Mo                                   | do                      | 67                                           | 105          | 30                               | 40                              | 260 | 0.6    | 5.0 |
| 4Sn—12Mo                                   | do                      | 66                                           | 99           | 38                               | 43                              | 257 | 0      | 0   |
| 6Sn—15Mo                                   | do                      | 138                                          | 142          | 6                                | 34                              | 320 | 0      | 0   |
| 8Sn—8Mo                                    | do                      | 65                                           | 125          | 11                               | 13                              | 264 | 0      | —   |
| 8Sn—10Mo                                   | do                      | 38                                           | 100          | 20                               | 49                              | 312 | 0.5    | 0.5 |
| 8Sn—12Mo                                   | do                      | 94                                           | 109          | 15                               | 38                              | 253 | 0      | 0   |
| 10Sn—10Mo                                  | do                      | 43                                           | 126          | 11                               | 24                              | 247 | 0.4    | —   |
| 10Sn—10Mo                                  | do                      | 87                                           | 119          | 11                               | 46                              | 282 | 0.5    | 0.5 |
| 10Sn—12Mo                                  | do                      | 117                                          | 122          | 14                               | 37                              | 275 | 0      | 0   |
| 12Sn—8Mo                                   | do                      | 61                                           | 134          | 8                                | 13                              | 255 | 0      | —   |
| 12Sn—10Mo                                  | do                      | 89                                           | 124          | 9                                | 31                              | 262 | 0      | 1.4 |
| 12Sn—12Mo                                  | do                      | 117                                          | 122          | 14                               | 37                              | 290 | 0      | 0   |
| 14Sn—6Mo                                   | do                      | 41                                           | 137          | 11                               | 15                              | 266 | 0      | —   |
| 14Sn—10Mo                                  | do                      | 115                                          | 120          | 17                               | 50                              | 287 | 0      | 0   |
| 14Sn—12Mo                                  | do                      | 114                                          | 118          | 17                               | 45                              | 280 | 0      | 0   |
| 14Sn—12Mo                                  | do                      | 120                                          | 120          | 18                               | 28                              | 296 | 0      | —   |
| 14Sn—16Mo                                  | do                      | 119                                          | 121          | 9                                | 30                              | 270 | 0      | —   |
| 16Sn—8Mo                                   | do                      | 112                                          | 118          | 18                               | 36                              | 293 | 0      | —   |
| 16Sn—12Mo                                  | do                      | 123                                          | 124          | 11                               | 38                              | 279 | 0      | —   |
| 18Sn—8Mo                                   | do                      | 118                                          | 124          | 11                               | 36                              | 294 | 1.5    | —   |
| 5Sn—10Mo                                   | 1,380° F.—quenched      | 120                                          | 128          | 10                               | 22                              | —   | —      | —   |
| 5Sn—10Mo                                   | 1,380° F.—quenched+aged | 169                                          | 173          | 2                                | 7                               | —   | —      | —   |
| 5Sn—10Mo                                   | 1/2 hr. at 400° C.      | —                                            | —            | —                                | —                               | —   | —      | —   |
| 14Sn—10Mo                                  | 1,380° F.—quenched+aged | 187                                          | 182          | 5                                | 17                              | —   | —      | —   |
| 14Sn—10Mo                                  | 1 hr. at 500° C.        | —                                            | —            | —                                | —                               | —   | —      | —   |
| 14Sn—10Mo                                  | 1,380° F.—quenched+aged | 154                                          | 163          | 7                                | 13                              | —   | —      | —   |
| 14Sn—10Mo                                  | 16 hr. at 500° C.       | —                                            | —            | —                                | —                               | —   | —      | —   |

Table V below shows the effect of chromium additions to the titanium-tin base. The observed improvement is of the same general order of magnitude as for the molybdenum addition and hence requires no detailed comment.

and a titanium base of commercial purity, the addition of 2% iron increases the ultimate strength from 123,000 to 177,000 p.s.i. with substantially no change in ductility. At the 10% tin level, the ultimate strength is increased from 110,000 to 150,000 p.s.i. with no change in ductility

TABLE V  
Ti—Sn—Cr alloys  
[Annealed condition.]

| Composition, Percent<br>(Balance Titanium) |      |       | Tensile properties:<br>p.s.i. $\times 1,000$ |                      | Percent<br>Elonga-<br>tion<br>in 1" | Percent<br>Reduction<br>in Area | Vickers<br>Hard-<br>ness | Min.<br>Bend T |
|--------------------------------------------|------|-------|----------------------------------------------|----------------------|-------------------------------------|---------------------------------|--------------------------|----------------|
| Sn                                         | Cr   | Other | 0.2%<br>Offset<br>Yield                      | Ultimate<br>Strength |                                     |                                 |                          |                |
| IODIDE TITANIUM BASE                       |      |       |                                              |                      |                                     |                                 |                          |                |
| 5                                          | 2.5  | —     | 78                                           | 97                   | 12                                  | 31                              | 265                      | 1.6            |
| 10                                         | 2.5  | —     | 85                                           | 98                   | 10                                  | 39                              | 241                      | 1.4            |
| 15                                         | 2.5  | —     | 117                                          | 128                  | 7                                   | 25                              | 329                      | 1.1            |
| COMMERCIAL TITANIUM BASE                   |      |       |                                              |                      |                                     |                                 |                          |                |
| 1                                          | 4    | —     | 102                                          | 112                  | 19                                  | 55                              | 279                      | 0.5            |
| 5                                          | 4    | —     | 114                                          | 123                  | 19                                  | 53                              | 311                      | 1.0            |
| 5                                          | 10   | —     | 132                                          | 138                  | 13                                  | 45                              | 320                      | —              |
| 9                                          | 0.25 | —     | 70                                           | 90                   | 27                                  | 52                              | 298                      | 1.6            |
| 9                                          | 0.5  | —     | 81                                           | 104                  | 20                                  | 46                              | 301                      | 1.7            |
| 9                                          | 1.25 | —     | 88                                           | 101                  | 15                                  | 33                              | 301                      | 1.9            |
| 9                                          | 2.5  | —     | 117                                          | 128                  | 16                                  | 37                              | 328                      | 1.7            |
| 9                                          | 5    | —     | 52                                           | 120                  | 15                                  | 23                              | 299                      | 0.9            |
| 9                                          | 10   | —     | 129                                          | 130                  | 16                                  | 31                              | 330                      | 0.9            |
| 9                                          | 15   | —     | 143                                          | 146                  | 14                                  | 36                              | 353                      | 1.6            |
| 10                                         | 2    | —     | 123                                          | 130                  | 16                                  | 48                              | 328                      | 2.1            |
| 10                                         | 4    | —     | 131                                          | 138                  | 12                                  | 49                              | 335                      | 1.8            |
| 10                                         | 6    | —     | 140                                          | 143                  | 10                                  | 43                              | 338                      | 0.7            |
| 10                                         | 8    | —     | 141                                          | 148                  | 11                                  | 42                              | 336                      | 1.5            |
| 10                                         | 10   | —     | 144                                          | 153                  | 5                                   | 8                               | 431                      | Br             |
| 15                                         | 4    | —     | 151                                          | 156                  | 8                                   | 34                              | 386                      | 1.9            |
| 9                                          | 1.25 | 0.20  | 125                                          | 131                  | 17                                  | 42                              | 351                      | 1.9            |
| 9                                          | 0.25 | 0.20  | 133                                          | 139                  | 11                                  | 52                              | 349                      | 1.7            |
| 9                                          | 0.25 | 0.250 | 114                                          | 121                  | 28                                  | 56                              | 369                      | 1.1            |
| 9                                          | 0.5  | 0.250 | 114                                          | 125                  | 27                                  | 58                              | 368                      | 1.7            |
| 9                                          | 1.25 | 0.20  | 124                                          | 133                  | 14                                  | 40                              | 371                      | 2.5            |
| 9                                          | 2.5  | 0.20  | 135                                          | 145                  | 8                                   | 20                              | 380                      | 2.5            |
| 9                                          | 0.25 | 0.20  | 103                                          | 121                  | 27                                  | 43                              | 368                      | 2.4            |
| 9                                          | 0.5  | 0.20  | 112                                          | 132                  | 18                                  | 45                              | 356                      | 1.6            |
| 9                                          | 1.25 | 0.2N  | 136                                          | 147                  | 13                                  | 40                              | 386                      | 2.5            |
| 9                                          | 2.5  | 0.2N  | 138                                          | 144                  | 13                                  | 27                              | 393                      | 1.7            |
| 9                                          | 0.25 | 0.2N  | 109                                          | 128                  | 19                                  | 34                              | 355                      | 2.5            |
| 9                                          | 0.5  | 0.2N  | 106                                          | 128                  | 21                                  | 45                              | 362                      | 2.3            |

Table VI shows the effect of adding iron to the titanium-tin base. It will be noted by comparison with Table I that the iron addition tremendously increases the ultimate strength accompanied in general by retention of adequate ductility. With the 15% tin analysis

45 upon the addition of 4% iron. Here again, as in the previous data, the addition of the interstitials enhances the strength properties with no loss in ductility as can be seen by comparison of the 9% tin, 0.5% iron analyses:

TABLE VI  
Ti—Sn—Fe alloys  
[Annealed condition.]

| Composition, Percent<br>(Balance Titanium) |      |       | Tensile properties:<br>p.s.i. $\times 1,000$ |                      | Percent<br>Elonga-<br>tion<br>in 1" | Percent<br>Reduction<br>in Area | Vickers<br>Hard-<br>ness | Min.<br>Bend T |
|--------------------------------------------|------|-------|----------------------------------------------|----------------------|-------------------------------------|---------------------------------|--------------------------|----------------|
| Sn                                         | Fe   | Other | 0.2%<br>Offset<br>Yield                      | Ultimate<br>Strength |                                     |                                 |                          |                |
| IODIDE TITANIUM BASE                       |      |       |                                              |                      |                                     |                                 |                          |                |
| 5                                          | 2.5  | —     | 60                                           | 97                   | 12                                  | 17                              | 247                      | 1.0            |
| 10                                         | 2.5  | —     | 95                                           | 119                  | 8                                   | 19                              | 293                      | 1.9            |
| 15                                         | 2.5  | —     | 115                                          | 130                  | 6                                   | 15                              | 333                      | 3.0            |
| COMMERCIAL TITANIUM BASE                   |      |       |                                              |                      |                                     |                                 |                          |                |
| 1                                          | 2    | —     | 77                                           | 104                  | 16                                  | 42                              | 255                      | 1.3            |
| 4                                          | 5    | —     | 97                                           | 124                  | 17                                  | 27                              | —                        | 2.0            |
| 5                                          | 2    | —     | 120                                          | 125                  | 18                                  | 38                              | 328                      | 3.6            |
| 9                                          | 0.25 | —     | 74                                           | 95                   | 20                                  | 42                              | 278                      | 2.5            |
| 9                                          | 0.5  | —     | 74                                           | 99                   | 18                                  | 39                              | 294                      | 2.7            |
| 9                                          | 1.25 | —     | 96                                           | 112                  | 19                                  | 46                              | 320                      | 1.6            |
| 9                                          | 2.5  | —     | 120                                          | 132                  | 15                                  | 39                              | 349                      | 1.3            |
| 9                                          | 5    | —     | —                                            | 103                  | 0                                   | 0                               | 375                      | Br             |
| 9                                          | 7.5  | —     | —                                            | 115                  | 0                                   | 0                               | 382                      | Br             |

TABLE VI—Continued

| Composition, Percent<br>(Balance Titanium) |      |       | Tensile Properties:<br>p.s.i. $\times 1,000$ |                      | Percent<br>Elonga-<br>tion<br>in 1" | Percent<br>Reduc-<br>tion<br>in Area | Vickers<br>Hard-<br>ness | Min.<br>Bend T |
|--------------------------------------------|------|-------|----------------------------------------------|----------------------|-------------------------------------|--------------------------------------|--------------------------|----------------|
| Sn                                         | Fe   | Other | 0.2%<br>Offset<br>Yield                      | Ultimate<br>Strength |                                     |                                      |                          |                |
| COMMERCIAL TITANIUM BASE—Continued         |      |       |                                              |                      |                                     |                                      |                          |                |
| 10                                         | 1.5  | ---   | 108                                          | 120                  | 18                                  | 40                                   | 330                      | 1.8            |
| 10                                         | 2    | ---   | 121                                          | 132                  | 9                                   | 31                                   | 347                      | 1.5            |
| 10                                         | 3    | ---   | 133                                          | 147                  | 14                                  | 36                                   | 359                      | 2.0            |
| 10                                         | 4    | ---   | 137                                          | 150                  | 10                                  | 37                                   | 370                      | 1.6            |
| 10                                         | 5    | ---   | 185                                          | 190                  | 5                                   | 16                                   | 446                      | Br             |
| 10                                         | 7.5  | ---   | 176                                          | 179                  | 8                                   | 31                                   | 428                      | 6.1            |
| 15                                         | 2    | ---   | 170                                          | 177                  | 12                                  | 32                                   | 411                      | 2.3            |
| 9                                          | 0.25 | 0.25O | 113                                          | 119                  | 25                                  | 54                                   | 343                      | 2.5            |
| 9                                          | 0.25 | 0.20  | 106                                          | 122                  | 21                                  | 38                                   | 341                      | 2.3            |
| 9                                          | 0.25 | 0.1N  | 91                                           | 109                  | 21                                  | 36                                   | 304                      | 2.3            |
| 9                                          | 0.5  | 0.25O | 104                                          | 125                  | 24                                  | 50                                   | 388                      | 1.3            |
| 9                                          | 0.5  | 0.20  | 105                                          | 125                  | 16                                  | 40                                   | 321                      | 1.8            |
| 9                                          | 0.5  | 0.1N  | 91                                           | 105                  | 17                                  | 42                                   | 306                      | 2.4            |
| 9                                          | 1.25 | 0.2C  | 123                                          | 134                  | 17                                  | 27                                   | 362                      | 1.7            |
| 9                                          | 1.25 | 0.20  | 110                                          | 123                  | 17                                  | 42                                   | 383                      | 1.9            |
| 9                                          | 1.25 | 0.2N  | 128                                          | 142                  | 18                                  | 45                                   | 380                      | 1.7            |
| 9                                          | 2.5  | 0.2C  | 143                                          | 152                  | 18                                  | 50                                   | 396                      | 1.5            |
| 9                                          | 2.5  | 0.20  | 139                                          | 152                  | 15                                  | 41                                   | 408                      | 2.3            |
| 9                                          | 2.5  | 0.2N  | 153                                          | 164                  | 15                                  | 34                                   | 404                      | Br             |

Table VII below shows the effects of additions of the beta stabilizers vanadium, tungsten, columbium, tantalum, copper, zirconium, cobalt, and nickel to the titanium-tin base.

TABLE VII  
Ti—Sn base plus V, W, Cb, Ta, Cu, Zr, Co, Ni, Si, Be  
alloys

[Annealed condition unless otherwise indicated.]

| Composition, Percent<br>(Balance Titanium) | Tensile Properties:<br>p.s.i. $\times 1,000$ |                      | Percent<br>Elongation<br>in 1" | Percent<br>Reduction<br>in Area | Vickers<br>Hardness | MBR, T. |   |
|--------------------------------------------|----------------------------------------------|----------------------|--------------------------------|---------------------------------|---------------------|---------|---|
|                                            | 0.2% Offset<br>Yield                         | Ultimate<br>Strength |                                |                                 |                     | L       | T |

IODIDE TITANIUM BASE

|                 |     |     |    |    |     |   |     |
|-----------------|-----|-----|----|----|-----|---|-----|
| 10Sn—2.5V       | 78  | 97  | 10 | 16 | 276 | — | 0.5 |
| 10Sn—2.5W       | 84  | 106 | 7  | 36 | 258 | — | 0.6 |
| 10Sn—2.5Cb      | 54  | 76  | 16 | 47 | 268 | — | 1.1 |
| 10Sn—2.5Ta      | 68  | 81  | 12 | 53 | 259 | — | 1.7 |
| 5Sn—1Cu         | 55  | 72  | 19 | 32 | 269 | — | 3.1 |
| 10Sn—1Cu        | 75  | 94  | 15 | 29 | 276 | — | 2.0 |
| 15Sn—1Cu        | 100 | 112 | 9  | 29 | 322 | — | 2.9 |
| 10Sn—1Cu—0.2O   | 98  | 108 | 22 | 38 | 340 | — | 1.9 |
| 10Sn—1Cu—0.2O   | 94  | 108 | 14 | 37 | 347 | — | 3.4 |
| 10Sn—1Cu—0.2N   | 114 | 128 | 11 | 28 | 375 | — | 0.3 |
| 10Sn—2.5Zr      | 94  | 110 | 20 | 40 | 270 | — | 2.2 |
| 10Sn—2.5Zr—0.2O | 108 | 117 | 18 | 43 | 356 | — | 2.1 |
| 10Sn—2.5Zr—0.2O | 99  | 113 | 18 | 42 | 318 | — | 3.7 |
| 10Sn—2.5Zr—0.2N | 129 | 136 | 15 | 39 | 369 | — | 3.3 |
| 10Sn—2.5Co      | 123 | 138 | 1  | 9  | 312 | — | 5.7 |
| 10Sn—2.5Ni      | 98  | 121 | 2  | 14 | 327 | — | 2.0 |

COMMERCIAL PURITY TITANIUM BASE

|                        |     |     |    |    |     |     |     |
|------------------------|-----|-----|----|----|-----|-----|-----|
| 10Sn                   | 86  | 98  | 18 | 52 | 281 | —   | 2.5 |
| 5Sn—22.5V <sup>1</sup> | 97  | 114 | 9  | 25 | 344 | 2.8 | 2.8 |
| 10Sn—1.5V              | 99  | 108 | 17 | 46 | 307 | —   | 2.6 |
| 10Sn—3V                | 125 | 136 | 15 | 41 | 333 | —   | 3.7 |
| 10Sn—5V                | 115 | 129 | 11 | 29 | 304 | —   | 1.6 |
| 10Sn—10V               | 107 | 112 | 7  | 40 | 258 | —   | 0   |
| 10Sn—15V               | 95  | 102 | 8  | 30 | 243 | —   | 0.7 |
| 0.5Sn—30V              | 106 | 109 | 9  | 25 | 254 | —   | 0   |
| 0.5Sn—40V              | 109 | 113 | 13 | 31 | 250 | —   | 0   |
| 10Sn—1W                | 108 | 114 | 17 | 47 | 333 | —   | 2.6 |
| 10Sn—2.5W              | 112 | 123 | 14 | 48 | 339 | —   | 2.7 |
| 10Sn—5W                | 118 | 145 | 15 | 43 | 360 | —   | 2.7 |
| 10Sn—10W               | 129 | 152 | 7  | 13 | 370 | —   | 5.0 |
| 10Sn—15W               | 146 | 174 | 4  | 8  | 363 | —   | 5.7 |
| 0.5Sn—30Cb             | 72  | 90  | 19 | 28 | 206 | —   | 0   |
| 5Sn—16Cb               | 64  | 90  | 15 | 32 | 228 | 0.8 | 1.0 |
| 5Sn—24Cb               | 43  | 100 | 10 | 22 | 235 | 1.3 | 2.9 |
| 10Sn—2.5Cb             | 92  | 102 | 21 | 51 | 304 | —   | 1.8 |
| 10Sn—5Cb               | 116 | 123 | 17 | 51 | 327 | —   | 2.6 |
| 10Sn—10Cb              | 120 | 130 | 10 | 39 | 312 | —   | 2.6 |
| 3Sn—4Cu <sup>2</sup>   | 68  | 88  | 15 | 34 | 243 | 1.8 | 1.3 |
| 6Sn—4Cu <sup>2</sup>   | 78  | 87  | 20 | 46 | 277 | 2.1 | 1.3 |
| 6Sn—6Cu                | 83  | 98  | 9  | 13 | 273 | 1.9 | 1.5 |
| 6Sn—8Cu                | 95  | 107 | 16 | 19 | 273 | 1.8 | 1.5 |
| 9Sn—4Cu                | 87  | 103 | 14 | 35 | 285 | 1.5 | 1.8 |
| 10Sn—0.5Cu             | 94  | 109 | 20 | 42 | 333 | —   | 1.6 |
| 10Sn—1Cu               | 87  | 104 | 16 | 34 | 289 | —   | 2.5 |
| 10Sn—2.5Cu             | 96  | 106 | 18 | 43 | 325 | —   | 2.6 |
| 10Sn—5Cu               | 122 | 131 | 13 | 24 | 342 | —   | 3.6 |
| 10Sn—7Cu <sup>3</sup>  | 108 | 128 | 10 | 24 | 300 | 1.5 | 1.5 |
| 11Sn—6Cu <sup>4</sup>  | 112 | 122 | 11 | 32 | 290 | 1.8 | 1.9 |

TABLE VII—Continued

| Composition, Percent<br>(Balance Titanium) | Tensile Properties:<br>p.s.i. $\times 1,000$ |                      | Percent<br>Elongation<br>in 1" | Percent<br>Reduction<br>in Area | Vickers<br>Hardness | MBR, T |     |
|--------------------------------------------|----------------------------------------------|----------------------|--------------------------------|---------------------------------|---------------------|--------|-----|
|                                            | 0.2% Offset<br>Yield                         | Ultimate<br>Strength |                                |                                 |                     | L      | T   |
| COMMERCIAL PURITY TITANIUM BASE—Continued  |                                              |                      |                                |                                 |                     |        |     |
| 12Sn-3Cu <sup>1</sup>                      | 94                                           | 110                  | 11                             | 28                              | 295                 | 1.9    | 1.9 |
| 12Sn-4Cu <sup>1</sup>                      | 94                                           | 109                  | 11                             | 24                              | 294                 | 2.9    | 2.9 |
| 12Sn-5Cu <sup>1</sup>                      | 106                                          | 118                  | 11                             | 33                              | 285                 | 2.0    | 2.0 |
| 14Sn-3Cu <sup>1</sup>                      | 124                                          | 136                  | 3                              | 14                              | 337                 | 2.9    | —   |
| 15Sn-4Cu <sup>1</sup>                      | 128                                          | 145                  | 11                             | 7                               | —                   | —      | —   |
| 18Sn-4Cu <sup>1</sup>                      | 142                                          | 151                  | 10                             | 25                              | —                   | —      | —   |
| 0.5Sn-30Ta <sup>2</sup>                    | 66                                           | 101                  | 14                             | 36                              | 220                 | —      | 0.2 |
| 5Sn-16Ta <sup>2</sup>                      | 80                                           | 98                   | 24                             | 53                              | 284                 | 1.2    | 1.2 |
| 5Sn-24Ta <sup>2</sup>                      | 72                                           | 110                  | 14                             | 35                              | 288                 | 1.6    | 1.6 |
| 10Sn-2.5Ta <sup>2</sup>                    | 85                                           | 95                   | 20                             | 51                              | 270                 | —      | 1.8 |
| 10Sn-5Ta <sup>2</sup>                      | 86                                           | 98                   | 21                             | 51                              | 283                 | —      | 1.7 |
| 10Sn-10Ta <sup>2</sup>                     | 110                                          | 111                  | 14                             | 48                              | 309                 | —      | 2.2 |
| 10Sn-1.0Co <sup>2</sup>                    | 90                                           | 106                  | 19                             | 39                              | 289                 | —      | 2.7 |
| 10Sn-2.5Co <sup>2</sup>                    | 108                                          | 125                  | 11                             | 22                              | 317                 | —      | 2.6 |
| 10Sn-5Co <sup>2</sup>                      | 111                                          | 124                  | 3                              | 7                               | 357                 | —      | Br  |
| 10Sn-1Ni <sup>2</sup>                      | 88                                           | 102                  | 18                             | 41                              | 283                 | —      | 1.8 |
| 10Sn-2.5Ni <sup>2</sup>                    | 95                                           | 111                  | 10                             | 31                              | 294                 | —      | 2.6 |
| 10Sn-5Ni <sup>2</sup>                      | 111                                          | 131                  | 11                             | 18                              | 327                 | —      | 5.7 |
| 0.5Sn-30Zr <sup>2</sup>                    | 115                                          | 145                  | 3                              | 3                               | 316                 | —      | 5.8 |
| 10Sn-1Zr <sup>2</sup>                      | 78                                           | 96                   | 23                             | 52                              | 285                 | —      | 1.6 |
| 10Sn-2.5Zr <sup>2</sup>                    | 84                                           | 100                  | 19                             | 50                              | 289                 | —      | 1.8 |
| 10Sn-5Zr <sup>2</sup>                      | 89                                           | 105                  | 18                             | 46                              | 309                 | —      | 2.5 |
| 10Sn-10Zr <sup>2</sup>                     | 93                                           | 108                  | 19                             | 46                              | 312                 | —      | 5.2 |
| 10Sn-0.5Si <sup>2</sup>                    | 100                                          | 111                  | 17                             | 46                              | 325                 | —      | 1.5 |

<sup>1</sup> 1,600° F. quenched.<sup>2</sup> 8 hrs. at 1,400° F.<sup>3</sup> 16 hrs. at 1,400° F.

Table VIII below shows the effects of adding a multiplicity of beta promoters to the titanium-tin base.

TABLE VIII

Mechanical properties of Ti-Sn base alpha-beta alloys containing two beta stabilizers (commercial purity titanium base)

[Annealed condition.]

| Composition, Percent (Balance Titanium) | Tensile properties:<br>p.s.i. $\times 1,000$ |                      | Percent<br>Elongation<br>in 1" | Percent<br>Reduction<br>in Area | Vickers<br>Hardness | Min. Bend Radius |     |
|-----------------------------------------|----------------------------------------------|----------------------|--------------------------------|---------------------------------|---------------------|------------------|-----|
|                                         | 0.2%<br>Offset<br>Yield                      | Ultimate<br>Strength |                                |                                 |                     | L                | T   |
| 10Sn-1.5Fe <sup>1</sup>                 | 108                                          | 120                  | 18                             | 40                              | 330                 | 1.8              | 3.0 |
| 10Sn-3Fe <sup>1</sup>                   | 133                                          | 147                  | 14                             | 36                              | 359                 | 2.0              | 4.8 |
| 10Sn-1.5Fe-4.5Mn <sup>1</sup>           | 145                                          | 151                  | 11                             | 32                              | 365                 | 1.7              | 5.9 |
| 10Sn-1.5Fe-2.5Mo <sup>1</sup>           | 126                                          | 139                  | 13                             | 30                              | 343                 | 2.7              | 5.6 |
| 10Sn-1.5Fe-2.5Cr <sup>1</sup>           | 127                                          | 143                  | 11                             | 34                              | 337                 | 2.8              | 5.2 |
| 10Sn-1.5Fe-2.5W <sup>1</sup>            | 120                                          | 131                  | 12                             | 32                              | 334                 | 2.6              | 5.2 |
| 10Sn-1.5Fe-5Cb <sup>1</sup>             | 129                                          | 141                  | 17                             | 32                              | 337                 | 2.6              | 4.6 |
| 10Sn-1.5Fe-5Ta <sup>1</sup>             | 121                                          | 134                  | 14                             | 43                              | 344                 | 2.6              | 5.2 |
| 10Sn-1.5Fe-5V <sup>1</sup>              | 123                                          | 133                  | 15                             | 25                              | 317                 | 0.6              | 4.2 |
| 10Sn-1.5Fe-2Ni <sup>1</sup>             | 110                                          | 120                  | 2                              | 5                               | 317                 | Br               | Br  |
| 10Sn-1.5Fe-2Co <sup>1</sup>             | 130                                          | 148                  | 9                              | 20                              | 366                 | Br               | Br  |
| 4Sn-3Fe-2Cu <sup>1</sup>                | 92                                           | 118                  | 18                             | 21                              | —                   | 1.0              | —   |
| 10Sn-1.5Fe-2.5Cu <sup>1</sup>           | 117                                          | 132                  | 11                             | 26                              | 357                 | 2.0              | 5.0 |
| 10Sn-3Fe-7.5Mo <sup>1</sup>             | 133                                          | 136                  | 10                             | 50                              | 303                 | 0                | 0   |
| 3Sn-3Fe-3Cr <sup>1</sup>                | 100                                          | 127                  | 17                             | 23                              | —                   | 1.0              | —   |
| 4Sn-5Cr-3Fe <sup>1</sup>                | 127                                          | 143                  | 22                             | 37                              | —                   | 0.6              | —   |
| 10Sn-3Fe-7.5Cr <sup>1</sup>             | 140                                          | 143                  | 14                             | 47                              | 321                 | 0                | 0   |
| 10Sn-4Fe-10Mo <sup>1</sup>              | 142                                          | 144                  | 10                             | 42                              | 325                 | 0                | 6.0 |
| 10Sn-4Fe-10Cr <sup>1</sup>              | 172                                          | 173                  | 0                              | 8                               | 375                 | Br               | Br  |
| 9Sn-2.5Mn <sup>1</sup>                  | 107                                          | 118                  | 11                             | 46                              | 336                 | 1.2              | 1.6 |
| 10Sn-5Mn <sup>1</sup>                   | 135                                          | 144                  | 12                             | 25                              | 375                 | 1.4              | Br  |
| 10Sn-2.5Mn-1.5Fe <sup>1</sup>           | 146                                          | 155                  | 11                             | 34                              | 359                 | 2.1              | 6.8 |
| 10Sn-2.5Mn-2.5Mo <sup>1</sup>           | 141                                          | 142                  | 1                              | 12                              | 340                 | 1.8              | 6.2 |
| 10Sn-2.5Mn-2.5Cr <sup>1</sup>           | 143                                          | 148                  | 13                             | 35                              | 364                 | 1.7              | 5.0 |
| 10Sn-2.5Mn-2.5W <sup>1</sup>            | 140                                          | 143                  | 8                              | 45                              | 351                 | 2.6              | 6.2 |
| 10Sn-2.5Mn-5Cb <sup>1</sup>             | 133                                          | 140                  | 12                             | 45                              | 354                 | 1.7              | Br  |
| 10Sn-2.5Mn-5Ta <sup>1</sup>             | 135                                          | 139                  | 12                             | 45                              | 350                 | 3.7              | 2.5 |
| 10Sn-2.5Mn-5V <sup>1</sup>              | 145                                          | 147                  | 7                              | 27                              | 344                 | 1.5              | Br  |
| 10Sn-2.5Mn-2Ni <sup>1</sup>             | 125                                          | 137                  | 6                              | 10                              | 346                 | Br               | Br  |
| 10Sn-2.5Mn-2Co <sup>1</sup>             | 147                                          | 153                  | 9                              | 34                              | 354                 | 4.1              | Br  |
| 5Sn-12Mn-1Cu <sup>1</sup>               | 143                                          | 146                  | 10                             | 45                              | 360                 | —                | —   |
| 10Sn-2.5Mn-2Cu <sup>1</sup>             | 129                                          | 136                  | 7                              | 37                              | 331                 | 1.9              | Br  |
| 3Sn-3Mn-3Fe <sup>1</sup>                | 116                                          | 141                  | 16                             | 19                              | —                   | 1.0              | —   |
| 10Sn-4Mn-3Fe <sup>1</sup>               | 144                                          | 150                  | 9                              | 34                              | 332                 | 0                | 0   |
| 10Sn-4Mn-7.5Mo <sup>1</sup>             | 125                                          | 127                  | 16                             | 52                              | 299                 | 0                | 0   |
| 6Sn-6Mn-9Cr <sup>1</sup>                | 134                                          | 135                  | 17                             | 56                              | 327                 | 0.1              | —   |
| 5Sn-7.5Mn-7.5Cr <sup>1</sup>            | 134                                          | 135                  | 16                             | 57                              | 351                 | 0.3              | —   |
| 10Sn-4Mn-7.5Cr <sup>1</sup>             | 140                                          | 143                  | 18                             | 39                              | 320                 | 0                | 0   |
| 10Sn-6Mn-4Fe <sup>1</sup>               | 146                                          | 152                  | 8                              | 25                              | 359                 | 3.0              | 4.3 |
| 10Sn-6Mn-10Mo <sup>1</sup>              | 141                                          | 142                  | 12                             | 38                              | 319                 | 0.2              | 0.8 |
| 10Sn-4.5Mn <sup>1</sup>                 | 132                                          | 142                  | 13                             | 32                              | 370                 | 1.5              | 4.0 |
| 10Sn-7Mn <sup>1</sup>                   | 143                                          | 147                  | 9                              | 35                              | 385                 | 1.2              | 4.6 |
| 10Sn-4.5Mn-2.5Mo <sup>1</sup>           | 147                                          | 149                  | 8                              | 25                              | 340                 | 2.3              | 4.8 |
| 10Sn-4.5Mn-2.5Cr <sup>1</sup>           | 147                                          | 153                  | 8                              | 26                              | 350                 | 1.4              | 5.4 |
| 10Sn-4.5Mn-2.5W <sup>1</sup>            | 137                                          | 144                  | 10                             | 33                              | 361                 | 0.5/2.3          | 4.7 |
| 10Sn-4.5Mn-5Cb <sup>1</sup>             | 135                                          | 143                  | 8                              | 21                              | 340                 | 1.5              | 4.8 |

TABLE VIII—Continued

| Composition, percent (Balance Titanium) | Tensile properties:<br>p.s.i. $\times 1,000$ |                      |                                | Vickers<br>Hardness | Min. Bend Radius |         |
|-----------------------------------------|----------------------------------------------|----------------------|--------------------------------|---------------------|------------------|---------|
|                                         | 0.2%<br>Offset<br>Yield                      | Ultimate<br>Strength | Percent<br>Elongation<br>in 1" |                     | L                | T       |
| 10Sn-4.5Mn-5Ta                          | 141                                          | 148                  | 8                              | 342                 | 1.9              | 4.6     |
| 10Sn-4.5Mn-5V                           | 135                                          | 142                  | 13                             | 327                 | 1.0              | 2.3/4.7 |
| 10Sn-4.5Mn-2Ni                          | 133                                          | 146                  | 2                              | 346                 | Br               | Br      |
| 10Sn-4.5Mn-2Co                          | 149                                          | 157                  | 9                              | 387                 | 1.9              | 6.1     |
| 10Sn-4.5Mn-2.5Ou                        | 139                                          | 149                  | 10                             | 351                 | 1.5              | 4.8     |
| 9Sn-2.5Mo                               | 96                                           | 113                  | 16                             | 299                 | 1.7              | 2.5     |
| 9Sn-5Mo                                 | 104                                          | 116                  | 14                             | 313                 | 1.7              | 3.5     |
| 10Sn-2.5Mo-2.5Cr                        | 127                                          | 138                  | 13                             | 333                 | 1.7              | 6.6     |
| 10Sn-2.5Mo-2.5W                         | 122                                          | 137                  | 12                             | 333                 | 4.1              | Br      |
| 10Sn-2.5Mo-5Cb                          | 122                                          | 132                  | 2                              | 331                 | 3.0              | 5.0     |
| 10Sn-2.5Mo-5Ta                          | 125                                          | 134                  | 10                             | 334                 | 2.5/4.0          | Br      |
| 10Sn-2.5Mo-5V                           | 117                                          | 122                  | 8                              | 297                 | 2.6              | 7.0     |
| 10Sn-2.5Mo-2Ni                          | 104                                          | 105                  | 11                             | 317                 | 2.4              | 7.0     |
| 10Sn-2.5Mo-2Co                          | 133                                          | 138                  | 3                              | 360                 | 1.6/3.2          | 4.9     |
| 10Sn-2.5Mo-2Cu                          | 117                                          | 124                  | 15                             | 330                 | 2.0              | 2.0     |
| 10Sn-7.5Mo-7Cr                          | 136                                          | 138                  | 15                             | 319                 | 0                | 0.4     |
| 10Sn-2.5Cr                              | 120                                          | 128                  | 17                             | 320                 | 2.0              | 2.5     |
| 10Sn-5Cr                                | 135                                          | 140                  | 11                             | 336                 | 1.5              | 3.5     |
| 10Sn-2.5Cr-2.5W                         | 123                                          | 129                  | 7                              | 339                 | 2.5              | 4.9     |
| 10Sn-2.5Cr-5Cb                          | 118                                          | 124                  | 12                             | 319                 | 2.0              | 2.5     |
| 10Sn-2.5Cr-5Ta                          | 126                                          | 134                  | 11                             | 317                 | 2.5              | 4.9/6.8 |
| 5Sn-6.5Cr-7.5V                          | 133                                          | 142                  | 9                              | 28                  | 1.2              | —       |
| 10Sn-2.5Cr-5V                           | 116                                          | 129                  | 12                             | 319                 | 0.9              | 2.6     |
| 10Sn-2.5Cr-2Ni                          | 121                                          | 139                  | 4                              | 335                 | 7.0              | Br      |
| 10Sn-2.5Cr-2Co                          | 148                                          | 156                  | 16                             | 387                 | 1.5              | 4.7     |
| 4Sn-6Cr-1.5Ou                           | 140                                          | 153                  | 11                             | 23                  | 0.9              | —       |
| 10Sn-2.5Cr-2.5Cu                        | 118                                          | 131                  | 13                             | 322                 | 1.5              | 6.5     |
| 10Sn-2.5W                               | 112                                          | 123                  | 14                             | 339                 | 2.7              | 2.7     |
| 10Sn-5W                                 | 118                                          | 145                  | 15                             | 360                 | 2.7              | 5.3     |
| 10Sn-2.5W-5Cb                           | 119                                          | 129                  | 16                             | 319                 | 2.6              | 5.0     |
| 10Sn-2.5W-5Ta                           | 120                                          | 129                  | 15                             | 336                 | 2.6/5.0          | 5.0     |
| 10Sn-2.5W-3V                            | 137                                          | 140                  | 10                             | 33                  | 2.8              | 6.2     |
| 10Sn-2.5W-2Ni                           | 108                                          | 124                  | 10                             | 325                 | 5.6              | 5.2     |
| 10Sn-2.5W-2Ou                           | 124                                          | 142                  | 14                             | 363                 | 2.4              | 4.7     |
| 10Sn-2.5W-2.5Ou                         | 116                                          | 123                  | 11                             | 342                 | 5.0              | 5.0     |
| 10Sn-5Cb                                | 116                                          | 123                  | 17                             | 327                 | 2.6              | 2.6     |
| 10Sn-10Cb                               | 120                                          | 130                  | 10                             | 39                  | 312              | 2.6     |
| 10Sn-5Cb-5Ta                            | 118                                          | 129                  | 13                             | 37                  | 329              | 2.6     |
| 10Sn-5Cb-5V                             | 113                                          | 119                  | 11                             | 34                  | 274              | 2.2     |
| 10Sn-5Cb-2Ni                            | 114                                          | 125                  | 10                             | 330                 | 2.8              | Br      |
| 10Sn-5Cb-2Co                            | 130                                          | 140                  | 13                             | 348                 | 1.5              | 1.5     |
| 10Sn-5Cb-2.5Ou                          | 121                                          | 130                  | 16                             | 327                 | 2.5/4.0          | 4.9     |
| 10Sn-5Ta                                | 86                                           | 98                   | 21                             | 51                  | 283              | 1.7     |
| 10Sn-10Ta                               | 110                                          | 111                  | 14                             | 48                  | 309              | 2.8     |
| 10Sn-5Ta-5V                             | 112                                          | 120                  | 11                             | 38                  | 281              | 2.3     |
| 10Sn-5Ta-2Ni                            | 91                                           | 106                  | 18                             | 37                  | 304              | 3.4     |
| 10Sn-5Ta-2Co                            | 103                                          | 125                  | 7                              | 325                 | Br               | Br      |
| 10Sn-5Ta-2.5Ou                          | 94                                           | 105                  | 16                             | 317                 | 2.4              | 2.8     |
| 10Sn-5V                                 | 108                                          | 118                  | 10                             | 39                  | 289              | 1.8     |
| 10Sn-10V                                | 107                                          | 112                  | 7                              | 40                  | 258              | 0       |
| 10Sn-5V-2Ni                             | 137                                          | 148                  | 6                              | 38                  | 339              | 4.8     |
| 10Sn-5V-2Ou                             | 122                                          | 134                  | 13                             | 31                  | 319              | 0.8     |
| 10Sn-5V-2.5Ou                           | 114                                          | 124                  | 6                              | 21                  | 304              | 1.5     |
| 10Sn-2Mn                                | 93                                           | 110                  | 16                             | 35                  | 300              | 2.0     |
| 10Sn-4Ni                                | 110                                          | 130                  | 12                             | 20                  | 320              | 5.0     |
| 10Sn-2Ni-2Ou                            | 97                                           | 118                  | 12                             | 27                  | 325              | 4.9     |
| 10Sn-2Ni-2.5Ou                          | 107                                          | 124                  | 18                             | 27                  | 342              | 4.0     |
| 10Sn-2Co                                | 105                                          | 120                  | 14                             | 30                  | 305              | 2.5     |
| 10Sn-4Co                                | 110                                          | 125                  | 5                              | 10                  | 350              | 5.0     |
| 10Sn-2Co-2.5Ou                          | 114                                          | 136                  | 5                              | 8                   | 339              | Br      |
| 10Sn-2.5Ou                              | 98                                           | 106                  | 18                             | 43                  | 325              | 2.6     |
| 10Sn-5Ou                                | 122                                          | 131                  | 13                             | 24                  | 342              | 2.6     |
| 10Sn-2.67Mn-2Fe-5Mo                     | 135                                          | 136                  | 7                              | 42                  | 312              | 0.2     |
| 10Sn-2.67Mn-2Fe-5Cr                     | 138                                          | 141                  | 9                              | 35                  | 315              | 0       |
| 10Sn-2.67Mn-5Mo-5Cr                     | 131                                          | 131                  | 15                             | 48                  | 310              | 0       |
| 10Sn-2Fe-5Mo-5Ou                        | 135                                          | 136                  | 16                             | 47                  | 312              | 0       |
| 10Sn-2Mn-1.5Fe-3.75Cr-3.75Mo            | 132                                          | 134                  | 14                             | 44                  | 310              | 0       |
| 5Sn-7.5Mn-7.5Cr-0.2Ou                   | 144                                          | 146                  | 14                             | 30                  | 357              | 5.2     |
| 5Sn-8Mn-4Cr-4Mo                         | 121                                          | 138                  | 19                             | 52                  | 357              | 0.2     |
| 4Sn-5Cr-5V-5Mn                          | 131                                          | 137                  | 14                             | 36                  | 357              | 1.3     |
| 4Sn-3Cr-2.5Mo-1.5Ou                     | 137                                          | 146                  | 13                             | 44                  | 300              | 1.0     |
| 4Sn-4Cr-2Fe-2Ou                         | 130                                          | 141                  | 19                             | 40                  | 357              | 0.7     |
| 4Sn-1Mn-2.5Cr-1Fe-1Cu-2Mo-0.5V          | 124                                          | 138                  | 21                             | 38                  | 357              | 0.9     |

<sup>1</sup> The tensile strength was reached before the 0.2% offset yield strength.<sup>2</sup> Defective sample.

From the test results of Tables II to VIII, inc., the following general conclusions may be drawn with respect to the effect of single and multiple beta stabilizer additions to the titanium-tin base. The beta isomorphous elements V, Cb, Ta, Mo and Zr alone or in combination with each other, produce alloys having similar properties. These alloys have medium strengths, good ductility, good thermal stability and, as shown below, are generally ductile as welded. The elements Fe, Cr and Mn which form systems containing sluggish eutectoid reactions, produce alloys which have high strengths, good ductility, fair thermal stability and are generally brittle as welded, except for low alloy contents of such additions. The elements with rapidly transforming eutectoids, Co, Ni, Cu and W, produce alloys which have medium

strengths, acceptable tensile ductility with borderline bend ductilities, poor thermal stability, and with the exception of the Ti-10Sn-5W alloy are intrinsically brittle as welded, except for extremely low additions of such elements. On the other hand, by judicious selection and combination of the beta promoters from one of the groups above mentioned with those of the other groups, multiple beta stabilizer alloys may be produced which combine the good qualities imparted by the elements from the groups selected, while tending to suppress and minimize their undesirable qualities. Thus, for example, the combination of beta isomorphous elements with the sluggish eutectoid elements results in alloys that have improved thermal stability and weld ductility as compared to those made with the sluggish eutectoid elements

alone. On the other hand, the test data shows that combinations of beta isomorphous elements with the rapid eutectoid elements do not result in improved thermal

properties of additions of the alpha stabilizer antimony to the titanium-tin base, with and without additions of the interstitials carbon, oxygen and nitrogen:

TABLE IX  
Ti—Sn base plus Sb alloys  
[Annealed condition.]

| Composition, Percent (Balance Titanium) |      |   |   |     | Tensile Properties: p.s.i. $\times 1,000$ |                   | Percent Elongation in 1" | Percent Reduction in Area | VHN | Min. Bend T |     |
|-----------------------------------------|------|---|---|-----|-------------------------------------------|-------------------|--------------------------|---------------------------|-----|-------------|-----|
| Sn                                      | Sb   | O | O | N   | 0.2 Percent Offset Yield                  | Ultimate Strength |                          |                           |     |             |     |
| IODIDE TITANIUM BASE                    |      |   |   |     |                                           |                   |                          |                           |     |             |     |
| 5                                       | 1    | — | — | —   | 22                                        | 37                | 61                       | 58                        | 88  | 0           |     |
| 10                                      | —    | — | — | —   | 52                                        | 68                | 23                       | 51                        | 210 | 1.6         |     |
| 10                                      | —    | — | — | 0.2 | 74                                        | 86                | 16                       | 39                        | 254 | 2.2         |     |
| 10                                      | —    | — | — | —   | 107                                       | 110               | 22                       | 55                        | 335 | 1.6         |     |
| 10                                      | —    | — | — | —   | 93                                        | 105               | 17                       | 36                        | 330 | 2.3         |     |
| 10                                      | —    | — | — | —   | 102                                       | 121               | 12                       | 37                        | 360 | 1.9         |     |
| 15                                      | 1    | — | — | —   | —                                         | 97                | 105                      | 14                        | 34  | 304         | 3.5 |
| COMMERCIAL PURITY TITANIUM BASE         |      |   |   |     |                                           |                   |                          |                           |     |             |     |
| 2.5                                     | 7.5  | — | — | —   | 76                                        | 96                | 16                       | 46                        | 268 | 2.1         |     |
| 2.5                                     | 12.5 | — | — | —   | 109                                       | 117               | 14                       | 42                        | 311 | 1.9         |     |
| 5                                       | 5    | — | — | —   | 74                                        | 94                | 17                       | 46                        | 262 | 1.5         |     |
| 5                                       | 10   | — | — | —   | 100                                       | 111               | 17                       | 44                        | 317 | 2.5         |     |
| 5                                       | 12.5 | — | — | —   | 116                                       | 125               | 9                        | 18                        | 331 | 2.3         |     |
| 5                                       | 15   | — | — | —   | —                                         | 126               | 0                        | 0                         | 354 | Br          |     |
| 7.5                                     | 2.5  | — | — | —   | 81                                        | 98                | 18                       | 43                        | 270 | 2.2         |     |
| 10                                      | 1    | — | — | —   | 79                                        | 94                | 21                       | 48                        | 292 | 2.3         |     |
| 10                                      | 2.5  | — | — | —   | 90                                        | 101               | 18                       | 47                        | 304 | 1.5         |     |
| 10                                      | 5    | — | — | —   | 107                                       | 116               | 17                       | 39                        | 325 | 1.7         |     |
| 10                                      | 7.5  | — | — | —   | 114                                       | 120               | 17                       | 47                        | 333 | 2.7         |     |
| 10                                      | 10   | — | — | —   | 125                                       | 133               | 16                       | 38                        | 342 | 4.9         |     |
| 10                                      | 12.5 | — | — | —   | —                                         | 114               | 0                        | 0                         | 348 | Br          |     |
| 12.5                                    | 2.5  | — | — | —   | 109                                       | 118               | 14                       | 36                        | 313 | 2.9         |     |
| 15                                      | 5    | — | — | —   | 128                                       | 135               | 17                       | 40                        | 333 | 3.6         |     |
| 15                                      | 7.5  | — | — | —   | 145                                       | 152               | 9                        | 26                        | 346 | 2.3         |     |
| 17.5                                    | 5    | — | — | —   | —                                         | 134               | 0                        | 6                         | 338 | 5.2         |     |

stability or weld ductility, and the same is generally true for combinations of sluggish eutectoid with rapid eutectoid elements. Over-all analysis of the test results indicates that for maximum thermal stability and weld ductility, the order of merit of the beta stabilizing elements is as follows: Cb, Mo, Ta, V, Cr, Mn, Fe, W, Cu, Co and Ni.

The following Table IX shows the effect on mechanical

40 Thus it will be seen by a comparison of Tables I and IX that antimony has about the same strengthening effect as an equivalent weight of tin and may be substituted therefor without undue embrittlement within the range of proportions set forth in the above table in column 20.

The following Table X shows the effect on mechanical properties of additions of the alpha stabilizers bismuth, indium, cadmium, silver, thallium, lead and zinc to the titanium-tin base:

TABLE X  
Ti—Sn base plus In, Bi, Pb, Ag, Cd, Tl and Zn alloys  
[Annealed condition.]

| Composition, Percent (Balance Titanium) |            | Tensile Properties: p.s.i. $\times 1,000$ |                   | Percent Elongation in 1" | Percent Reduction in Area | Vickers Hardness | Min. Bend T |
|-----------------------------------------|------------|-------------------------------------------|-------------------|--------------------------|---------------------------|------------------|-------------|
| Sn                                      | Other      | 0.2% Offset Yield                         | Ultimate Strength |                          |                           |                  |             |
| IODIDE TITANIUM BASE                    |            |                                           |                   |                          |                           |                  |             |
| 5                                       | —          | 27                                        | 43                | 40                       | 61                        | 105              | 0           |
| 5                                       | IBI        | 56                                        | 73                | 26                       | 37                        | 235              | 1.6         |
| 5                                       | IBI        | 50                                        | 66                | 30                       | 44                        | 190              | 1.2         |
| 10                                      | IBI        | 76                                        | 88                | 16                       | 40                        | 261              | 2.1         |
| 15                                      | IBI        | 95                                        | 106               | 18                       | 40                        | 312              | 2.2         |
| 10                                      | IBI—0.2O   | 103                                       | 107               | 18                       | 51                        | 324              | 1.6         |
| 10                                      | IBI—0.2O   | 94                                        | 106               | 16                       | 45                        | 338              | 2.0         |
| 10                                      | IBI—0.2N   | 117                                       | 123               | 20                       | 41                        | 356              | 1.7         |
| 10                                      | 2.5In      | 75                                        | 88                | 13                       | 43                        | 256              | 2.1         |
| 10                                      | 2.5In—0.2O | 101                                       | 108               | 20                       | 54                        | 337              | 2.0         |
| 10                                      | 2.5In—0.2O | 93                                        | 108               | 16                       | 46                        | 322              | 2.5         |
| 10                                      | 2.5In—0.2N | 109                                       | 119               | 18                       | 44                        | 350              | 2.8         |
| 10                                      | 1Cd        | 55                                        | 71                | 18                       | 54                        | 248              | 1.5         |
| 5                                       | 1Ag        | 53                                        | 71                | 22                       | 43                        | 191              | 1.3         |
| 10                                      | 1Ag        | 59                                        | 78                | 21                       | 39                        | 241              | 2.1         |
| 15                                      | 1Ag        | 91                                        | 103               | 16                       | 46                        | 308              | 2.3         |
| 10                                      | 1Ag—0.2O   | 102                                       | 104               | 19                       | 54                        | 321              | 2.4         |
| 10                                      | 1Ag—0.2O   | 93                                        | 105               | 16                       | 45                        | 322              | 3.5         |
| 10                                      | 1Ag—0.2N   | 133                                       | 139               | 12                       | 45                        | 386              | 6.3         |
| 10                                      | 2.5Tl      | 60                                        | 75                | 22                       | 57                        | 238              | 1.9         |

21  
TABLE X—Continued

| Composition, Percent (Balance Titanium) |        | Tensile Properties: psi. $\times 1,000$ |                   |    | Percent Elongation in 1" | Percent Reduction in Area | Vickers Hardness | Min. Bend T |
|-----------------------------------------|--------|-----------------------------------------|-------------------|----|--------------------------|---------------------------|------------------|-------------|
| Sn                                      | Other  | 0.2% Offset Yield                       | Ultimate Strength |    |                          |                           |                  |             |
| <b>COMMERCIAL PURITY TITANIUM BASE</b>  |        |                                         |                   |    |                          |                           |                  |             |
| 5                                       | ---    | 49                                      | 76                | 24 | 44                       | 197                       | 1.3              |             |
| 5                                       | ---    | 71                                      | 90                | 14 | 42                       | 246                       | 1.5              |             |
| 10                                      | 1Bi*   | 82                                      | 97                | 20 | 48                       | 297                       | 1.5              |             |
| 10                                      | 2.5Bi* | 86                                      | 99                | 17 | 45                       | 297                       | 2.4              |             |
| 10                                      | 5Bi*   | 87                                      | 101               | 19 | 48                       | 312                       | 1.5              |             |
| 10                                      | 2.5Bi* | 50                                      | 74                | 24 | 49                       | 206                       | 1.1              |             |
| 10                                      | 1In    | 79                                      | 94                | 25 | 61                       | 233                       | 1.7              |             |
| 10                                      | 2.5In  | 88                                      | 101               | 21 | 48                       | 297                       | 1.5              |             |
| 10                                      | 5In    | 92                                      | 104               | 17 | 49                       | 289                       | 1.9              |             |
| 10                                      | 10In   | 102                                     | 111               | 20 | 45                       | 325                       | 2.7              |             |
| 10                                      | 10Cd   | 79                                      | 92                | 18 | 41                       | 270                       | 1.8              |             |
| 10                                      | 1Ag    | 80                                      | 96                | 17 | 48                       | 252                       | 1.7              |             |
| 10                                      | 2.5Ag  | 82                                      | 95                | 18 | 47                       | 287                       | 1.5              |             |
| 10                                      | 5Ag    | 87                                      | 102               | 19 | 51                       | 309                       | 1.7              |             |
| 10                                      | 10Ag   | 91                                      | 104               | 18 | 45                       | 309                       | 2.5              |             |
| 10                                      | 10Pb*  | 87                                      | 101               | 23 | 47                       | 314                       | 2.3              |             |
| 10                                      | 10Zn*  | 73                                      | 86                | 22 | 52                       | 268                       | 1.6              |             |

\* Considerable weight loss occurred during melting.

Table XI below shows the effects of additions of the various compound formers to the titanium-tin base:

tendency to become embrittled as a result of welding. As further shown in said application, beta-containing alloys

22  
TABLE XI  
Alloys of Ti—Sn base plus compound formers Si, Be, Ce, B, Te, etc.  
[Annealed condition.]

| Composition, Percent (Balance Titanium) |        | Tensile Properties: psi. $\times 1,000$ |                   |    | Percent Elongation in 1" | Percent Reduction in Area | Vickers Hardness | Min. Bend T |
|-----------------------------------------|--------|-----------------------------------------|-------------------|----|--------------------------|---------------------------|------------------|-------------|
| Sn                                      | Other  | 0.2% Off. Set Yield                     | Ultimate Strength |    |                          |                           |                  |             |
| <b>IODIDE TITANIUM BASE</b>             |        |                                         |                   |    |                          |                           |                  |             |
| 10                                      | ---    | 85                                      | 99                | 20 | 36                       | 298                       | 1.5              |             |
| 10                                      | 1Ce    | 87                                      | 75                | 16 | 34                       | 250                       | 2.0              |             |
| 10                                      | 1Te    | 61                                      | 78                | 17 | 48                       | 232                       | 2.7              |             |
| 10                                      | 2.5Te  | 72                                      | 88                | 7  | 26                       | 242                       | 1.1              |             |
| 10                                      | 0.5B   | 54                                      | 72                | 21 | 38                       | 236                       | 1.8              |             |
| 10                                      | 2.5Th  | 60                                      | 75                | 22 | 57                       | 288                       | 1.9              |             |
| 10                                      | 1Si    | 80                                      | 97                | 16 | 38                       | 305                       | 1.6              |             |
| 10                                      | 0.2Be  | 70                                      | 90                | 12 | 22                       | 273                       | 1.6              |             |
| <b>COMMERCIAL PURITY TITANIUM BASE</b>  |        |                                         |                   |    |                          |                           |                  |             |
| 10                                      | 1Ce*   | 91                                      | 110               | 11 | 36                       | 298                       | 1.5              |             |
| 10                                      | 1Ce*   | 80                                      | 94                | 17 | 39                       | 285                       | 2.4              |             |
| 10                                      | 2.5Ce* | 78                                      | 92                | 15 | 33                       | 276                       | 3.2              |             |
| 10                                      | 0.5Si  | 100                                     | 110               | 17 | 45                       | 325                       | 1.5              |             |
| 10                                      | 1Si    | 97                                      | 109               | 17 | 35                       | 330                       | 5.0              |             |
| 10                                      | 2Si    | 104                                     | 108               | 3  | 8                        | 333                       | 7.0              |             |

\* Considerable weight loss occurred during melting.

The welding characteristics of the various types of alloys of the present invention, are described, and the weldable alloys thereof, covered by the above-mentioned co-pending joint application of the applicants Jaffee and Ogden herein, Serial No. 585,177. As therein shown, the all-alpha or substantially all-alpha titanium-tin base alloys of the present invention, containing up to about 16% tin, are weldable without serious impairment of ductilities, substantially throughout the entire range of analyses that such alloys are ductile in the cast or wrought condition. The same is shown in said application to be generally true with respect to the beta or mixed alpha-beta titanium-tin alloys obtained by additions of beta-promoters of the beta-isomorphous group, i.e., Mo, V, Cr, Ta and Zr, although certain of the molybdenum-containing analyses may require a post welding heat treatment as described in said application, for offsetting a

60 formed by additions of the sluggishly eutectoid beta promoters, Cr, Mn and Fe, are generally productive of brittle welds when present in substantial amounts, i.e., about 2-3%, although certain of the higher alloy analyses restricted to Cr and/or Mn additions are ductile as welded or can have their ductilities restored by post welding heat treatment as above mentioned, i.e., those containing up to about 7-8% Mn or up to about 18% Cr. The beta alloys formed by additions of Co, Ni, Cu and W having rapidly transforming eutectoids are intrinsically brittle in the welded condition when these additions are present in excess of about 2 to 3%, i.e., their ductilities cannot be restored by post welding heat treatment. The compound formers likewise impart intrinsic brittleness as welded to the titanium-tin base alloy when present in amounts exceeding about 2 to 3%.

70 Our investigations have established that the alloys in

accordance with the invention containing about 10 to 15% tin are wholly contamination resistant at temperatures up to 1050° C. and probably higher regardless of the type of alloy, i.e., whether all-alpha, mixed alpha-beta or all-beta. They have further established that there is a marked or critical reduction in contamination resistance commencing at about 5% tin as compared to that of the same alloy containing no tin. The tin-addition produces free scaling alloys in most cases, but this tendency to free scaling appears to be reduced when large quantities of beta stabilizers are present.

The findings above stated are based on the test results set forth in the following Table XII, the data for which was obtained by arc melting 15-gram buttons of each of the compositions indicated in the table, including the tin-free alloy bases. The buttons were forged at 850° C. to about  $\frac{3}{8}$ " square x  $1\frac{1}{4}$ " long. Each forged billet was then descaled and sectioned into two samples. One sample was heated in air for four hours at 1050° C. and furnace cooled. The second sample received the same treatment in argon. These samples were furnace cooled to minimize any heat treatment effects that might have occurred with some of the alloys during cooling from the beta field. Weight-change data, scale appearance, thickness after wire brushing off the loose scale, and hardness penetration data were obtained for each specimen, with results as recorded in the table.

TABLE XII

*Oxidation test data for Ti—Sn base alloys containing Ta, W, Cb, W, Mo, Fe, Cr or Mn*

[Condition: 4 hr. at 1050° C. in air and furnace cooled.]

| Composition, percent<br>(Balance Titanium) | Weight<br>Gain<br>g./dm. <sup>3</sup> | Metal-<br>Thickness<br>Loss,<br>Mils | Depth of<br>Contam-<br>ination,<br>Mils | Increase<br>in VHN<br>5 Mils<br>Below<br>Surface |
|--------------------------------------------|---------------------------------------|--------------------------------------|-----------------------------------------|--------------------------------------------------|
| 100Ti                                      | 3.5                                   | 10                                   | 60                                      | 240                                              |
| 5Sn                                        | 15.5                                  | 18                                   | 40                                      | 60                                               |
| 10Sn                                       | 13.5                                  | 19                                   | NiI                                     | NiI                                              |
| 15Sn                                       | 11.9                                  | 18                                   | NiI                                     | NiI                                              |
| 5Ta                                        | 2.00                                  | NiI                                  | 80                                      | 350                                              |
| 5Sn—5Ta                                    | 6.49                                  | NiI                                  | 55                                      | 200                                              |
| 10Sn—5Ta                                   | 16.09                                 | 21                                   | 30                                      | 60                                               |
| 15Sn—5Ta                                   | 19.41                                 | 28                                   | NiI                                     | NiI                                              |
| 2.5W                                       | 3.52                                  | 1                                    | 80                                      | 220                                              |
| 5Sn—2.5W                                   | 23.80                                 | 36                                   | 40                                      | 60                                               |
| 10Sn—2.5W                                  | 20.60                                 | 29                                   | 30                                      | 30                                               |
| 15Sn—2.5W                                  | 12.27                                 | 11                                   | NiI                                     | NiI                                              |
| 5eB                                        | 1.66                                  | NiI                                  | 70                                      | 230                                              |
| 5Sn—5Cb                                    | 5.19                                  | NiI                                  | 40                                      | 150                                              |
| 10Sn—5Cb                                   | 14.30                                 | 20                                   | NiI                                     | NiI                                              |
| 15Sn—5Cb                                   | 18.67                                 | 26                                   | NiI                                     | NiI                                              |
| 5V                                         | 5.18                                  | 2                                    | 85                                      | 300                                              |
| 5Sn—5V                                     | 12.33                                 | 15                                   | 35                                      | 50                                               |
| 10Sn—5V                                    | 14.88                                 | 18                                   | NiI                                     | NiI                                              |
| 15Sn—5V                                    | 18.70                                 | 35                                   | NiI                                     | NiI                                              |
| 2.5Mo                                      | 2.8                                   | 2                                    | 80                                      | 280                                              |
| 5Sn—2.5Mo                                  | 5.0                                   | 22                                   | 40                                      | 50                                               |
| 10Sn—2.5Mo                                 | 20.9                                  | 32                                   | 10                                      | 50                                               |
| 15Sn—2.5Mo                                 | 20.9                                  | 30                                   | 20                                      | 40                                               |
| 15Mo                                       | 3.8                                   | 4                                    | 20                                      | 80                                               |
| 5Sn—15Mo                                   | 12.7                                  | 21                                   | 15                                      | 50                                               |
| 10Sn—15Mo                                  | 12.4                                  | 22                                   | NiI                                     | NiI                                              |
| 15Sn—15Mo                                  | 15.5                                  | 21                                   | 20                                      | 50                                               |
| 2.5Fe                                      | 3.8                                   | 3                                    | 120                                     | 280                                              |
| 5Sn—2.5Fe                                  | 12.0                                  | 16                                   | 25                                      | 80                                               |
| 10Sn—2.5Fe                                 | 10.7                                  | 18                                   | 50                                      | 30                                               |
| 15Sn—2.5Fe                                 | 8.5                                   | 14                                   | NiI                                     | 20                                               |
| 7.5Fe                                      | 3.7                                   | 2                                    | 80                                      | 250                                              |
| 5Sn—7.5Fe                                  | 6.6                                   | 9                                    | 35                                      | 50                                               |
| 10Sn—7.5Fe                                 | 9.4                                   | 14                                   | NiI                                     | NiI                                              |
| 15Sn—7.5Fe                                 | 7.5                                   | 6                                    | NiI                                     | 90                                               |
| 2.5Cr                                      | 4.6                                   | 0.5                                  | 60                                      | 280                                              |
| 5Sn—2.5Cr                                  | 9.9                                   | 7                                    | 80                                      | 140                                              |
| 10Sn—2.5Cr                                 | 6.6                                   | 10                                   | NiI                                     | NiI                                              |
| 15Sn—2.5Cr                                 | 12.8                                  | 24                                   | NiI                                     | NiI                                              |
| 10Cr                                       | 3.5                                   | 0.5                                  | 40                                      | 300                                              |
| 5Sn—10Cr                                   | 3.5                                   | 0.5                                  | NiI                                     | NiI                                              |
| 10Sn—10Cr                                  | 4.8                                   | 8                                    | NiI                                     | NiI                                              |
| 15Sn—10Cr                                  | 3.1                                   | 6                                    | NiI                                     | NiI                                              |
| 2.5Mn                                      | 3.0                                   | 2                                    | 80                                      | 300                                              |
| 5Sn—2.5Mn                                  | 12.1                                  | 18                                   | 5                                       | 100                                              |
| 10Sn—2.5Mn                                 | 14.9                                  | 21                                   | NiI                                     | 20                                               |
| 15Sn—2.5Mn                                 | 12.8                                  | 20                                   | NiI                                     | NiI                                              |
| 7.5Mn                                      | 3.7                                   | 2                                    | 80                                      | 250                                              |
| 5Sn—7.5Mn                                  | 6.6                                   | 9                                    | 40                                      | 50                                               |
| 10Sn—7.5Mn                                 | 9.4                                   | 14                                   | NiI                                     | NiI                                              |
| 15Sn—7.5Mn                                 | 7.5                                   | 6                                    | NiI                                     | NiI                                              |

As above stated, the majority of the specimens were found to be free scaling, but the Ti—(5-15)Sn—10Cr alloys had rather adherent scales with little loss in metal by oxidation and no noticeable contamination as measured by hardness. The Ti—10Cr control alloy had a similar scale, but the underlying metal was highly contaminated. Thus, when 10% chromium is present, tin appears to afford the contamination resistance without the free scaling characteristics, thus indicating utility of these alloys at elevated temperatures.

Our investigations have further shown that the Ti—(5-15)Sn—10Cr alloy, with and without additions of up to 5% of one or more of iron, molybdenum and manganese, have excellent elevated temperature hardnesses combined with contamination resistance at temperatures as high as 800° to 900° F., and good hardness at temperatures up to 1100° to 1200° F. This is shown by the test results submitted in the following Table XIII.

TABLE XIII

*Hot hardness values of Ti—Sn base alloys for elevated temperature service*

| Composition,<br>Percent (Balance<br>Titanium) | [As hot rolled and annealed] |        |        |        |          |          |          |       |
|-----------------------------------------------|------------------------------|--------|--------|--------|----------|----------|----------|-------|
|                                               | 80 F.                        | 250 F. | 500 F. | 750 F. | 1,000 F. | 1,250 F. | 1,500 F. | 80 F. |
| 100Ti                                         | 219                          | 195    | 141    | 116    | 72       | 33       | —        | 233   |
| 5Sn**                                         | 240                          | 221    | 163    | 133    | 107      | 60       | 23       | 287   |
| 10Sn**                                        | 270                          | 235    | 189    | 152    | 132      | 71       | 27       | 292   |
| 10Cr                                          | 306                          | 276    | —      | 223    | 123      | 32       | 18       | 476   |
| 15Cr                                          | 297                          | 235    | 269    | 247    | 160      | 51       | 27       | 357   |
| 5Sn—10Cr                                      | 355                          | 294    | 261    | 235    | 144      | 42       | 24       | 359   |
| 10Sn—10Cr                                     | 326                          | 313    | 275    | 254    | 180      | 55       | 26       | 339   |
| 5Sn—15Cr                                      | 360                          | 327    | 279    | 265    | 179      | 58       | 32       | 377   |
| 5Sn—10Cr—5Fe                                  | 389                          | 353    | 322    | 315    | 244      | 92       | 37       | 409   |
| 5Sn—10Cr—5Mo                                  | 315                          | 290    | 246    | 240    | 190      | 75       | 33       | 346   |
| 5Sn—10Cr—5Mn                                  | 324                          | 314    | 286    | 271    | 186      | 68       | 31       | 376   |
| 8Mn                                           | 377                          | 340    | 269    | 235    | 106      | 46       | —        | —     |

\*Hardness at room temperature after being heated to 1,500° F.

\*\*Annealed 2 hours at 850° C. prior to testing; other analyses annealed at 700° C.

Referring to the above data, a comparison of the hardness values of the binary Ti—Sn alloys with the binary Ti—Cr alloys shows that it is the chromium or beta addition which promotes the higher hardness at temperatures up to 800° to 900° F. As further shown by the above data, the combination of tin and chromium provides an added hardening increment, due to the tin, which is maintained at elevated temperatures. As further shown, the substitution of manganese, iron and molybdenum for part of the chromium, has varied effects. Iron additions result in higher hardnesses, which prevail at temperatures up to about 1200° F. Manganese additions do not change the hardness of the Ti—Sn—Cr alloy, while molybdenum additions produce some decrease in hardness which prevails at all temperatures referred to. On the basis of hardness alone, the Ti—5Sn—10Cr—5Fe alloy is best. However, on the basis of strong and ductile room temperature properties as well as elevated temperature contamination resistance and hardness, the Ti—Sn—Cr—(Mo, Mn) alloys are of best all-around utility.

The room temperature properties of these alloys are given in the following Table XIV:

TABLE XIV

*Mechanical properties of Ti—Sn—Cr base alloys for elevated temperature service*

[These alloys were 980° C. forged, hot rolled at 1,400° F. to 0.080 inch, descaled, hot rolled at 1,300° F. to 0.040 inch, held 15 minutes at 1,800° F., furnace cooled at 1,100° F., and air cooled to room temperature]

| Composition, Percent<br>(Balance Titanium) | Tensile Properties:<br>p.s.i.×1,000 |                      | Percent<br>Elonga-<br>tion<br>in 1" | Percent<br>Reduc-<br>tion<br>in Area | Vickers<br>Hard-<br>ness | Minimum<br>Bend<br>Radius, T |       |
|--------------------------------------------|-------------------------------------|----------------------|-------------------------------------|--------------------------------------|--------------------------|------------------------------|-------|
|                                            | 0.2% Off-<br>set Yield              | Ultimate<br>Strength |                                     |                                      |                          | L                            | T     |
| 10Cr-----                                  | 126                                 | 134                  | 10                                  | 46                                   | 300                      | 0                            | 1.5   |
| 5Sn—10Cr-----                              | 132                                 | 138                  | 13                                  | 45                                   | 320                      | 0.9                          | 5.5   |
| 10Sn—10Cr-----                             | 145                                 | 151                  | 2                                   | 7                                    | 372                      | -----                        | ----- |
| 5Sn—10Cr—5Fe-----                          | 165                                 | 168                  | 2                                   | 6                                    | 373                      | Br                           | Br    |
| 5Sn—10Cr—5Mo-----                          | 134                                 | 139                  | 11                                  | 46                                   | 314                      | 0.9                          | 1.8   |
| 5Sn—10Cr—5Mn-----                          | 149                                 | 155                  | 7                                   | 15                                   | 382                      | Br                           | Br    |

The alloys of the invention may be made by melt casting in a cold mold, employing an electric arc in an inert atmosphere, or may be produced in other ways in which the alloy is rendered molten before casting.

Where the alloys are to be used in the form of sheets, the minimum bend ductilities may range as high as 20T, and where they are to be used in massive form, as in forgings, the percent tensile elongation may range as low as 1 or 2%. Minimum bend ductility T is defined as the minimum radius to which a specimen can be bent through an angle of 75° without fracture, expressed as a multiple of the specimen thickness.

It will be observed from the data in the tables above set forth that the alloys of the invention have ultimate tensile strengths at least 10% in excess of the unalloyed titanium base metal, and in the vast majority of instances,

ultimate strengths at least 30 to 50% in excess of the unalloyed titanium base metal.

What is claimed is:

A titanium base alloy consisting essentially of about: 0.5-23% tin, up to 1% carbon, up to 0.5% oxygen, up to 0.4% nitrogen, and 0.5-18% of at least one alpha promoter selected from the group consisting of antimony, indium, silver, cadmium, zinc, thallium, bismuth and lead, balance substantially titanium, characterized in having a tensile elongation of at least 2% and a tensile strength at least 10% in excess of that of the corresponding titanium-tin binary alloy.

References Cited in the file of this patent

UNITED STATES PATENTS

2,779,677 Jaffee et al. ----- Jan. 29, 1957